# EUROPEAN PATENT APPLICATION

(11) **EP 4 775 704 A1**
(43) Date of publication of application: **15.07.2026**
(21) Application number: 24861547.8
(22) Date of filing: 15.05.2024
(51) Int. Cl.: C22C 33/04, C21C 5/28, C22C 38/00

(54) **HIGH-PURITY HIGH-CARBON STEEL WIRE ROD AND PRODUCTION METHOD THEREFOR**

(30) Priority: 07.09.2023 CN 202311150761
(71) Applicant: Zhangjiagang Rongsheng Special Steel Co. Ltd., Suzhou, Jiangsu 215625 (CN); Institute of Research of Iron and Steel, Jiangsu Province/Sha-Steel, Co. Ltd (CN), Suzhou, Jiangsu 215625 (CN); Jiangsu Shagang Group Co., Ltd., Suzhou, Jiangsu 215625 (CN)
(72) Inventor: ZHAO, Jiaqi, Suzhou, Jiangsu 215624 (CN); CAI, Xiaofeng, Suzhou, Jiangsu 215624 (CN); LI, Qiang, Suzhou, Jiangsu 215624 (CN); MA, Jianchao, Suzhou, Jiangsu 215624 (CN); LI, Jie, Suzhou, Jiangsu 215624 (CN)
(74) Representative: Cleanthous, Marinos
(86) International application number: PCT/CN2024/093334
(87) International publication number: WO 2025/050698

(57) **Abstract**

The present invention belongs to the technical field of steelmaking. Disclosed are a high-purity high-carbon steel wire rod and a production method therefor. In addition to alloying elements and Fe, the high-purity high-carbon steel wire rod further comprises the following chemical components in mass percentage: C: 0.5-1.0%, P≤0.008%, S≤0.0025%, T.O≤0.0010%, N≤0.0020%, H≤0.0002%, Alt≤0.0010%, and Ti≤0.0005%. The production method comprises: hot-metal pretreatment, converter smelting, RH vacuum treatment, continuous casting of large billets, cogging and grinding, high-speed wire rolling, Stelmor air cooling, and obtainment of a finished wire rod. In the present invention, highly homogenized casting blanks and high-quality wire rods are obtained, and high-purity base materials are provided for high-end wire rod products. Provided in the present invention are a high-purity high-carbon steel wire rod and a production method therefor, which can be used for producing highly homogenized wire rod products having high cleanliness.

## Description

### TECHNICAL FIELD

The present disclosure relates to a high-purity high-carbon steel wire and a production method therefor, belonging to the technical field of steelmaking.

### BACKGROUND

High-purity high-carbon steel wire has extremely high technical requirements for impurity element content, inclusions, segregation, and the like, which are used in applications such as high-strength automotive suspension springs, cord steel, and bridge cable steel, directly affecting the fatigue life and drawing performance of products, which in turn affects the overall service life and safety of the applied equipment or engineering structures. To obtain a high-carbon steel wire product with high strength and high performance, it is necessary to improve the control level of impurity elements and inclusions during production, as well as enhance compositional uniformity, internal quality, and surface quality of a billet during continuous casting, thereby comprehensively improving the quality of the high-carbon steel wire products.

Spring, as an important basic component, is widely used in automobiles, machinery, railway and other fields. As a safety bearing component, the spring needs to bear high-cycle alternating load in service, and its failure mode is mainly fatigue fracture. A large number of studies show that for high-strength and high-cycle fatigue springs, impurity elements, large-sized inclusions, segregation and surface quality are main causes of fatigue failure. Cord steel, as a skeleton supporting material in automobile tire rubber, has extremely high requirements for its quality stability. Large-sized inclusions, segregation and abnormal microstructures are main reasons for drawing fracture and torsional stranding fracture, which seriously affects the quality stability of products and further affects operation safety of automobiles. Bridge cable steel is mainly used in large-scale bridge engineering, which is sensitive to phosphorus content, large-sized inclusions, segregation, network carbide, and the like. In the drawing process, brittle fracture or torsional fracture may be caused due to the foregoing defects, which affects the product quality and further affects the engineering quality and safety.

High-quality high-carbon steel wires, such as spring steel, cable steel, and cord steel, are generally produced by KR (Kanbara Reactor), converter, LF (Ladle Furnace) refining, VD/RH (Vacuum Degasser/Ruhrstahl-Heraeus), and continuous casting process, with a long production process. The KR is used for hot metal desulfurization; the converter is for decarburization and dephosphorization; converter tapping and LF refining are used for deoxidation, alloying, and slag formation; and VD/RH vacuum treatment is used for degassing and inclusion removal. Some manufacturers of spring steels employ an acidic slag system to control inclusions as low-melting-point calcium aluminosilicate inclusions. However, the acidic slag system causes severe erosion of refractory materials, which is prone to causing excessive exogenous inclusions, resulting in fatigue fracture of the spring and affecting the service performance. Due to the presence of Al in some cable steel grades, the inclusions are mainly calcium aluminosilicates and calcium aluminates, which exhibit a wide range of compositional fluctuations and poor control stability. As the product size is relatively large, drawing processes generally do not suffer from inclusion-induced fracture, but it is prone to fracture caused by large-sized inclusions during torsion. Cord steel is generally produced through KR, converter, LF refining, and continuous casting processes. An acidic slag system is employed to control the melting point of inclusions and improve drawing performance. However, the acidic slag system causes severe erosion of refractory materials, and exogenous brittle inclusions are a primary cause of drawing breakage in cord steel. In addition, large-sized and low-melting-point silicate inclusions may also lead to fracture during stranding and torsion of the cord steel, affecting the processing performance and quality stability of the product.

In patent No. 202110338648X, high-cleanliness spring steel and a production method therefor are provided. The spring steel is produced by hot metal deep desulfurization, converter dephosphorization, LF refining, RH vacuum and continuous casting, and the hot metal is desulfurized until an S content is ≤0.0015%, the molten steel with a P content of ≤0.011% is obtained by converter blowing, and converter tapping and bottom blowing during refining process are accurately controlled. Combined with RH vacuum treatment process and tundish induction heating technology, inclusions in the molten steel are controlled throughout the entire process to obtain a spring steel wire rod with high cleanliness. However, a high-basicity slag system which includes 55% to 60% of CaO and 20% to 25% of SiO2 is adopted. Due to high C and Si contents in the spring steel, under a high-basicity condition, Al₂O₃ in the slag or refractory material is reduced by element Si, resulting in the increase of alumina composition in molten steel inclusions, and the probability of the occurrence of high-melting-point aluminosilicate inclusions and brittle inclusions is greatly increased, which is unfavorable to the fatigue life control of the spring steel.

In Patent No. 2022101243433, a method for controlling brittle inclusions in cord steel is provided. The method employs slag with low basicity and moderate oxidizability for smelting, where the basicity ranges from 0.9 to 1.2, and the T.Fe+MnO content in the slag ranges from 2% to 5%. In addition, alloys with low aluminum content and refractory materials with low alumina content are selected for production, so that alumina and magnesia-alumina spinel inclusions in the molten steel can be effectively controlled, which is highly beneficial to the drawing performance of the cord steel wire rod. However, due to the selection of an acidic slag system, although alloys and refractory materials with low aluminum content are used, the slag has a certain degree of oxidizability, and the T.Fe+MnO content is significantly high, resulting in a high total oxygen content in the molten steel. This leads to increased erosion of refractory materials of the ladle and tundish during the smelting process. In addition to controlling the chemical composition of the refractory materials, it is also necessary to propose higher requirements on their physical properties such as strength and density. Otherwise, large-sized magnesia inclusions introduced into the molten steel due to refractory material erosion may cause drawing breakage in cord steel products.

In Patent No.202010061162.1, a method for controlling an ultra-low melting point plastic inclusion in cord steel is provided. By controlling an oxygen content in molten steel during tapping, a manganese alloy is first used for deoxidation, followed by the addition of an appropriate amount of carbon powder for auxiliary deoxidation. During refining, the elements Mn and C are first adjusted to meet the standards, and then a silicon alloy is added to adjust the Si content of the molten steel to the target composition. An ultra-low melting point SiO₂+MnO type inclusions are obtained by designing the deoxidation and alloying process. However, this technological solution employs a low-basicity acidic slag system, and utilizes Mn for pre-deoxidation, followed by Si for deoxidation, resulting in poor overall deoxidation efficiency of the molten steel. This leads to significant oxidation of carbon (C) in the refractory material, causing decarburization and erosion of the refractory material during steelmaking and continuous casting and an increase in a risk that refractory material particles enter the molten steel to cause excessive brittle inclusions. In addition, in the slag, a MnO content reaches 3% to 5% and SiO₂ content ranges from 40% to 50%, the slag further reacts with composition such as MgO and Al₂O₃ in the refractory material to form low-melting-point silicates, which exacerbates erosion of the refractory material and causes an increase in brittle inclusions or large-sized silicate inclusions in the molten steel.

In patent No.2013106819801, a spring steel wire production process for controlling inclusions is provided, including the following steps: (1) smelting according to an aluminum-free deoxidation process; (2) top-bottom combined blowing in a converter; (3) argon blowing treatment at an Ar station; (4) LF ladle argon-blowing refining, with a target basicity controlled at 0.7 to 2.0; (5) vacuum treatment; and (6) casting into a billet, followed by rolling into wire rod through a high-speed wire rod rolling process. Although this process employs aluminum-free deoxidation, the used low-basicity slag cannot effectively absorb silicate inclusions generated by Si/Mn deoxidation. In addition, the low-basicity slag system exacerbates erosion of a refractory material, which increases the number of exogenous inclusions introduced by the refractory material, such as alumina and magnesia-alumina spinel. Such inclusions are the most detrimental to fatigue life.

In patent No. 2012102042739, a spring steel wire rod and an inclusion control method thereof are provided. A process route is as follows: (1) converter tapping with high carbon content; (2) silicon-manganese deoxidation after converter tapping; (3) LF refining, controlling an endpoint oxygen content in the steel at 20 ppm to 40 ppm; (4) continuous casting with low superheat; and (5) continuous rolling and wire rod rolling. The inclusion in the steel has a width size not greater than 10 µm, and an aspect ratio greater than 3. However, this process has the disadvantage of a relatively high oxygen content (20 ppm to 40 ppm) in the steel, and an acid-soluble aluminum (Als) content in the molten steel is between 0.01% and 0.02%, which is easy to cause an increase in non-metallic brittle inclusions in the spring steel, leading to a significant negative impact on the fatigue life of the spring during service.

In patent No. 2016102603055, a smelting process for controlling inclusions in spring steel is provided, including: (1) electric arc furnace primary smelting; (2) argon blowing; (3) LF furnace refining; (4) VD furnace refining; and (5) continuous casting. An Si/Mn aluminum-free deoxidation process is used for pre-deoxidation in the electric arc furnace primary smelting process, and active lime, a composite agent and a refining slag are used at the same time. Although brittle inclusions in steel can be well controlled, the basicity of slag in the late refining period is controlled at 0.7-1.4, and an acidic slag seriously erodes the refractory material of a ladle and a continuous casting tundish, which is easy to cause foreign inclusions to exceed the standard.

In patent No. 2020111278482, a wire rod for 2300-MPa prestressed steel strand and a production method therefor are provided. The production of the wire rod undergoes the technological processes of hot metal pre-desulfurization, converter smelting, out-of-furnace refining, bloom continuous casting, cogging, high-speed wire-rod rolling, air cooling and a salt bath treatment in turn. A superheat of molten steel in a tundish during continuous casting is 12°C to 25°C, measures such as electromagnetic stirring and dynamic soft reduction are adopted to reduce solidification segregation, and a bloom two-heat rolling process is adopted, which is strongly cooled before phase transformation to inhibit the formation of network cementite. After the salt bath treatment, the wire rod structure has sorbite of ≥ 95% and network carbon of ≤1 grade. However, the adoption of low superheat casting is not conducive to the control of inclusion floating and cracks caused high reduction. The cast billet after rolling also needs to undergo salt bath treatment, leading to long overall process flow and high production cost.

In patent No. 2021110884598, a production method for a deep-drawn high-carbon steel wire rod is provided. The steel includes chemical composition as follows: 0.69% to 1.02% of C, 0.15% to 0.35% of Si, 0.40% to 0.90% of Mn, less than or equal to 0.35% of Cr, less than or equal to 0.025% of P, less than or equal to 0.025% of S, with the balance being iron and inevitable impurities. Special mold flux and a large-chamfered mold are used for continuous casting, a high temperature is used for high-speed wire rod heating, holding time is controlled, and an oxidizing atmosphere is used to increase a burning loss of billet surface in a reheating furnace, and the grade of the network cementite on the surface of wire rod is less than or equal to 0.5. However, the applicable high-carbon steel wire rod has high overall content in impurity elements such as P and S, and poor cleanliness. Employing a highly oxidizing atmosphere in the reheating furnace may cause severe surface decarburization of the billet, leading to the increase of grinding allowances and adverse impact on the production cost and wire rod quality control. This approach is unsuitable for the production of a high-quality high-carbon steel wire rod product.

In patent No. 2022109583109, a spring steel wire and a production method therefor are provided, involving hot metal desulfurization, converter smelting, LF refining, RH vacuum treatment, bloom continuous casting, cogging and grinding, high-speed wire rod rolling, and air cooling. During smelting, the alloy and slag composition, and the like are controlled, and the inclusions are controlled to be calcium aluminosilicate inclusions with 10% to 25% of Al₂O₃, 45% to 65% of SiO₂, and 15% to 30% of CaO. A reduction amount is controlled by dividing a solid fraction (fs) at the solidification center of the continuously cast billet into three ranges, thereby achieving the control of segregation in the cast billet. In addition, the internal and surface quality of the wire rod are controlled by controlling grinding, the atmosphere in a reheating furnace, a rolling process, and other factors, thereby improving the performance of the spring steel wire rod and the final products. However, the overall basicity of the slag is relatively high, and the inclusions are calcium aluminosilicate inclusions with 10% to 25% of Al₂O₃, 45% to 65% of SiO₂, and 15% to 30% of CaO, with a melting point of 1400°C to 1500°C. Although present as low-melting-point liquid inclusions at a molten steel temperature, these inclusions solidify at a rolling temperature and exhibit almost no deformation, which is detrimental to the control of spring fatigue performance. In addition, due to the use of a medium-basicity slag system with the basicity of 1.6 to 2.0, and high SiO₂ content in the inclusions of the molten steel, there is a certain degree of erosive effect on the refractory material, which may exacerbate the erosion of refractory material particularly during strong vacuum stirring. In addition, as there is no further limitations on the used refractory material and other auxiliary materials, the quality of the refractory material and other auxiliary materials cannot be controlled, and exogenous high-melting-point brittle inclusions may significantly affect the fatigue life of the springs. The three-segmented distributed reduction control is difficult to achieve accurate control of the reduction effect of the cast billet. In addition, as the billet is not protected by a coating, severe oxidation and decarburization occur on a surface layer of the billet in the reheating furnace. This requires extensive grinding to control the quality, which is unfavorable to both production efficiency and the stability of quality control.

High-grade high-carbon steel wire products for critical applications have strict requirements for impurity elements, inclusions, and composition and microstructure uniformity. Therefore, controlling the content of impurity elements, the type and size of inclusions, and the uniformity of composition and microstructure has always been a key focus in the research and development of the high-grade high-carbon steel wire rod. Analysis indicates that impurity elements primarily need to be controlled by limiting P and S to reduce quality problems such as cold brittleness and hot brittleness, and it is necessary to control the contents of Al, Ti, and N in the molten steel to prevent the formation of hard inclusions such as alumina, magnesia- alumina spinel, and titanium nitride. Inclusions formed from deoxidation products, slag-metal reactions and refractory spalling require control through both plasticity modification and size refinement. Meanwhile, it is also necessary to accurately control the uniformity of composition and microstructure and surface quality of the wire rod mainly through continuous casting and rolling processes. During continuous casting, the cast billet with high compositional uniformity is obtained by controlling the superheat of the molten steel, the intensity of cooling water, and reduction process, and the problems such as segregation, network carbides and surface quality are mitigated by combining cogging and grinding, controlled rolling and controlled cooling technologies. Therefore, a high-purity high-carbon steel wire rod can be obtained.

### SUMMARY

To solve the problems described above, the present disclosure provides high-purity high-carbon steel wire and a production method therefor, with specific technical solutions as follows.

A high-purity high-carbon steel wire is provided, where the high-purity high-carbon steel wire, in addition to alloying elements and Fe element, further includes the following chemical composition in mass percentage: 0.5% to 1.0% of C, less than or equal to 0.008% of P, less than or equal to 0.0025% of S, less than or equal to 0.0010% of T.O, less than or equal to 0.0020% of N, less than or equal to 0.0002% of H, less than or equal to 0.0010% of Alt, and less than or equal to 0.0005% of Ti.

Further, in the high-carbon steel wire rod, a mass content of inclusions other than those of the SiO₂-MnO type is ≤ 20%, a number density of inclusions larger than 1 µm is ≤3.5 particles/mm², and a number density of inclusions larger than 5 µm is ≤0.06 particles/mm²; the maximum transverse size of inclusions is ≤12 µm, longitudinal inclusions has a maximum width of ≤10 µm and a length of ≤25 µm; the size of brittle inclusions is ≤3 µm; a carbon segregation index of the cast billet is 0.95 to 1.05, and a carbon segregation index of the wire rod is ≤1.05.

A method for manufacturing a high-purity high-carbon steel wire, production is carried out according to the following technological processes: hot metal pretreatment, converter smelting, RH vacuum treatment, bloom continuous casting, cogging and grinding, high-speed wire-rod rolling, Stelmor air cooling, and finished wire rod obtaining, and the method specifically includes the following steps:
Step 1: carrying out KR hot metal pretreatment to low-sulfur hot metal, and charging the low-sulfur hot metal into a converter;
Step 2: carrying out converter smelting with a converter charge of 145±5 t and a hot metal ratio of 80% to 90%, where clean scrap is selected for smelting, and the converter adopts a double-slag dephosphorization process;
Step 3: during converter tapping, at the start of tapping, adding 30% to 40% of low-nitrogen carburizer into a ladle at first, and adding 20% to 30% of metallic manganese for pre-deoxidation, completing tapping after the added low-nitrogen carburizer and metallic manganese are fully dissolved into molten steel and no carbon powder particles float on the surface, and then adding silicon carbide and a synthetic slag to ladle slag surface in sequence to deoxidize the slag surface and form slag; and during converting tapping, maintaining ladle bottom blowing throughout the entire process, where in dual bottom blowing of the ladle, one porous plug has a maximum flow rate of 600 NL/min to 800 NL/min, and the other porous plug has a flow rate of 30% to 50% of the maximum flow rate, the two porous plugs are arranged on the bottom of the ladle at an angle of 135 degrees, located at a position 55% of a radius from the center of the ladle, and configured to blow argon into the molten steel to stir the molten steel and the slag;
upon completion of converter tapping, adding silicon carbide to deoxidize the ladle slag, with at an addition amount of 0.5 kg/t to 1.5 kg/t, and after the silicon carbide is added, adding a synthetic slag for slag formation, with an addition amount of 8 kg/t to 12 kg/t; controlling dual bottom blowing flow rates of the ladle at 150 NL/min to 250 NL/min after the synthetic slag is added, and transporting the ladle to RH for treatment after the synthetic slag is evenly spread;
Step 4: RH furnace refining, enabling a RH arrival temperature to be ≥1590°C, a C content to be ≥0.2%, an Mn content to be 0.15-0.35%, and an oxygen content to be ≤0.020%; during rapid evacuation treatment upon arrival at the RH station, controlling an operating pressure of the vacuum chamber to be ≤1 mbar, and the lift gas flow rate to be 150 Nm³/min to 200 Nm³/min; adding silicon carbide for deoxidation according to arrival composition, and controlling deep vacuum treatment time to be ≥15 min, taking a sample for composition test, and based on a composition test result and a composition requirement of a smelted steel grade, selecting one or more of low-nitrogen carburizer, ultra-pure silicon, metallic manganese, ferrochrome, and ferrovanadium for alloying; after the composition meets standards, reducing a pumping capacity of a RH vacuum system by 40% to 60%, increasing a pressure in a vacuum chamber, reducing a lift gas flow rate to 80 Nm³/min to 100 Nm³/min, and after carrying out net circulation for ≥5 min, breaking vacuum;
after vacuum breaking in RH, controlling soft stirring time to be ≥6 min, the maximum flow rate of one of the dual porous plugs to be 60 NL/min to 80 NL/min, and the flow rate of the other porous plug to be 40% to 50% of the maximum flow rate; and transporting the ladle to a continuous casting platform to stand for 10 min and more, and then starting casting;
Step 5: carrying out bloom continuous casting, where the bloom has a cross-section of 300 mm×390 mm, implementing protective casting throughout the entire continuous casting process, employing a low-basicity and low-alumina tundish covering flux, and controlling a superheat fluctuation of the molten steel in the tundish to be ≤5°C by using tundish electromagnetic induction heating equipment, where tundish induction heating is carried out with a current of 1500 A to 1800 A and a voltage of 1600 V to 2000 V; when a carbon content in the steel is 0.5%≤C<0.8%, controlling a superheat of the molten steel to be 20°C to 35°C; and when a carbon content in the steel is that 0.8%≤C<1.0%, controlling the superheat of the molten steel to be 30°C to 45°C, maintaining a tundish tonnage at 48±1 tons, and the tonnage during ladle change at 40 tons to 45 tons;
the mold electromagnetic stirring is carried out with a current of 450 A 650 A, a frequency of 6 Hz to 8 Hz, a mold water flow rate is set 2750 NL/min to 3050 NL/min, a secondary cooling segment water flow rate is set to 550 NL/min to 650 NL/min, and a mold level fluctuation is set to ≤2 mm; continuous casting is carried out at a constant casting speed, and the continuous casting speed is controlled at 0.6 m/min to 0.7 m/min; and
a solid fraction fs at the solidification center of a continuously cast billet is divided into four ranges, when 0.1≤fs<0.3, a reduction ratio accounts for 10% to 15%; when 0.3≤fs<0.5, a reduction ratio accounts for 20% to 30%; when 0.5≤fs<0.8, a reduction ratio accounts for 50% to 60%; when 0.8≤fs<1, a reduction ratio accounts for 10% to 20%; and a total reduction amount is controlled at 15 mm to 30 mm, thereby obtaining a cast billet with C segregation index of 0.95 to 1.05;
Step 6: carrying out cogging and grinding; and
Step 7: carrying out rolling and air cooling to control cooling intensity and improve structure and properties.

Further, step 2 includes the following steps: adopting intensive bottom-blowing stirring in an early stage of converter blowing, with a high lance position and a low oxygen flow rate, adopting a medium-basicity slag system with basicity of 1.8 to 2.2; adding pellets to control a T.Fe content in the slag to be ≥25%; stopping oxygen blowing upon completion of early-stage blowing, controlling a temperature to be 1380°C to 1430°C, carrying out bottom-blowing stirring for more than 3 min until a P content is ≤0.016%, followed by slag removal; after the slag removal is completed, continuing blowing with a low lance position and a high oxygen supply flow rate; adding lime to form a high-basicity slag system, and adding pellets to control a minimum T.Fe to be ≥15% during blowing; at the end of blowing, controlling the temperature to be ≥1650°C, the T.Fe content to be ≥25%, and the basicity to be ≥6; and carrying out slag removal at first, and upon completing the slag removal, tapping while retaining the slag with a slide gate.

Further, in step 6: during cogging and grinding, the continuously cast billet is heated in a cogging reheating furnace and undergoes soaking and heat preservation, a billet temperature is controlled to be 1100°C to 1200°C, and an initial rolling temperature is controlled to be 1040°C to 1180°C; a rolled billet is obtained after cogging and rolling; the rolled billet is subjected to magnetic particle inspection, followed by full surface grinding; and for a position with an apparent flaw detection defect on the surface, spot grinding is carried out additionally, with an average grinding depth of ≥0.5 mm; and
during coating spraying of the rolled billet, a high-temperature-resistant coating is sprayed onto the surface of the ground rolled billet, with a thickness of 0.3 mm to 1.5 mm.

Further, in a case of controlling an atmosphere in the reheating furnace, the rolled billet after coating spraying is heated in a steel-rolling reheating furnace and undergoes soaking and heat preservation, a temperature of the rolled billet in the steel-rolling reheating furnace is controlled at 1030°C to 1190°C, an initial rolling temperature is controlled at 910°C to 1170°C, a finish rolling entry temperature is controlled at 840°C to 960°C, and a finish rolling exit temperature is controlled at 990°C to 1050°C; and in percent by volume, a total content of H₂O and O₂ in atmosphere composition in the reheating furnace is ≤2.5%.

Further, in step 7, a rolled wire obtained in a high-speed wire rod rolling procedure is subjected to temperature-controlled air cooling, and a wire laying temperature of an air cooling line is controlled at 820°C to 925°C.

Further, a KR arrival temperature is ≥1380°C, and in the hot metal, an S content is ≤0.045%, a C content is 4.1% to 4.6%, an Si content is 0.25% to 0.60%, a Ti content is ≤0.03%, a P content is ≤0.11%, with the balancing being Fe and other inevitable impurity elements; upon arrival at a KR station, a blast furnace slag is skimmed off with a slag skimming rate of ≥95%; then, a desulfurizing agent is added for desulfurization, and after desulfurization, slag skimming is carried out again with a slag skimming rate of ≥95%; subsequently, the desulfurizing agent is added for the second desulfurization, with a slag skimming rate of ≥ 98%; and a KR departure temperature is controlled to be ≥1330°C, and a departure S content is controlled to be ≤0.0008%.

Further, the clean scrap used by the converter includes composition as follows: less than or equal to 0.015% of P, less than or equal to 0.0050% of S, less than or equal to 0.01% of Ti, and conventional elements such as C, Si, Al, Mn, Fe; and at the end of converter blowing, a C content is 0.03% to 0.07%, an O content is 0.035% to 0.075%, a P content is ≤0.008%, and a tapping weight of the converter is 135±5 t.

Further, the low-carbon nitrogen carburizer added during converter tapping includes less than or equal to 0.045% of N, with the balance being C and inevitable impurity elements;
the metallic manganese includes more than or equal to 99% of Mn, less than or equal to 0.003% of Ti, less than or equal to 0.005% of Al, less than or equal to 0.0065% of P, less than or equal to 0.0035% of S, with the balance being iron and inevitable impurity elements; and
the silicon carbide includes more than or equal to 98% of SiC, and other inevitable impurity elements.

The synthetic slag added during converter tapping includes composition as follows: 45% to 55% of CaO, 20% to 30% of SiO₂, 5% to 10% of CaF₂, 1% to 3% of MnO, less than or equal to 3% of MgO, less than or equal to 1.5% of Al₂O₃, and other inevitable impurity composition, and has a basicity of 1.5 to 2.0; and in phase composition, monocalcium silicate accounts for 35% to 45%, dicalcium silicate accounts for 15% to 25%, and the others are CaO, CaF₂, MnO, and inevitable phases.

Further, the low-carbon nitrogen carburizer added during RH vacuum treatment includes less than or equal to 0.045% of N, with the balance being C and inevitable impurity elements;
the metallic manganese includes more than or equal to 99% of Mn, less than or equal to 0.003% of Ti, less than or equal to 0.005% of Al, less than or equal to 0.0065% of P, less than or equal to 0.0035% of S, with the balance being iron and inevitable impurity elements; and
the silicon carbide includes more than or equal to 98% of SiC, and other inevitable impurity elements;
the ultra-pure silicone includes 80% to 85% of Si, less than or equal to 0.0035% of Al, less than or equal to 0.001% of Ti, less than or equal to 0.005% of P, less than or equal to 0.0025% of S, with the balance being iron and inevitable impurity elements;
the ferrochrome includes 55% to 60% of Cr, less than or equal to 1.8% of C, less than or equal to 0.006% of S, less than or equal to 0.013% of P, with the balance being iron and inevitable impurity elements; and
the ferrovanadium includes 45% to 50% of V, less than or equal to 1.6% of C, less than or equal to 0.005% of S, less than or equal to 0.012% of P, with the balance being iron and inevitable impurity elements.

Further, a ladle brick used in step 3 is a magnesia-carbon brick, which includes less than or equal to 3.0% of magnesium aluminate spinel, less than or equal to 3% of C, with the balance being inevitable impurity composition; and
a refractory material used for a dipping tube and a bottom tank of a RH vacuum furnace in step 4 is an ultra-low-carbon magnesite-chrome brick, which includes less than or equal to 1.5% of C, 85% to 95% of MgO, 5% to 12% of Cr₂O₃, less than or equal to 3.0% of magnesium aluminate spinel, and other inevitable impurity composition.

Further, in step 5, the low-basicity and low-alumina tundish covering flux for continuous casting includes main composition as follows: 40%-50% of CaO, 30% to 40% of /SiO₂, 3% to 6% of CaF₂, less than or equal to 2% of Al₂O₃, 3% to 6% of MgO, and other inevitable composition; and
a magnesia spraying material for an inner wall of the tundish includes composition as follows: more than or equal to 80% of MgO, 5% to 10% of CaO, 1% to 3% of SiO₂, and other inevitable composition.

Further, in step 5, an overall submerged entry nozzle is used for casting, an insertion depth of the submerged entry nozzle is 10 mm to 15 mm, a mold flux has a slag layer thickness of 10 mm to 20 mm and a consumption rate of 0.15 kg/ton to 0.25 kg/ton;
each of a stopper rod and the submerged entry nozzle is made of a magnesia carbon material, the stopper rod further includes the following composition in mass percentage: 80% to 85% of MgO, 8% to 12% of C, less than or equal to 1.5% of Al₂O₃, 1% to 4% of SiC, 2% to 3% of SiO₂, and other inevitable impurity composition; and
the submerged entry nozzle has an inner wall thickness of 5 mm to 7 mm, and includes the following composition in mass percentage: 75% to 80% of MgO, 6% to 10% of C, 3% to 5% of SiC, 5% to 10% of SiO₂, and other inevitable impurity composition.

Further, in step 6, a coating is sprayed for protection before the rolled billet enters the reheating furnace, where the coating has a thickness of 0.3 mm to 1.5 mm, and the high-temperature coating includes CaO, SiO₂, Al₂O₃, MgO, ZrO₂, C, as well as small amounts of alkali metal oxides, inorganic binders, and surfactants.

Further, the bloom is cogged into a billet with a cross-section of 140 mm×140 mm, and is subjected to flow inspection and grinding, heating in a reheating furnace, rolling, and controlled cooling on a Stelmor air-cooling line to obtain a wire rod that is free from surface defects such as a fold, a scab, and a scratch, and has no fully decarburization layer on surface thereof.

The present disclosure further claims a high-purity high-carbon steel wire prepared by the method provided by the present disclosure.

The present disclosure further claims a wire rod prepared from the high-purity high-carbon steel wire, where the wire rod includes a high-quality cord steel wire rod with a C content of ≤0.87% for drawing a fine wire with a diameter of 0.1 mm or more and a high-quality diamond wire rod with a C content is more than 0.87% and less than or equal to 1.0% for drawing a fine wire with a diameter of 0.05 mm or more.

The present disclosure further claims a 1600-2400 MPa grade spring steel and a 1800-2200 MPa grade cable steel prepared from the high-purity high-carbon steel wire.

Cord steel requires excellent drawing and stranding/twisting properties, spring steel needs high fatigue resistance, and cable steel requires high torsion properties of materials. Such high-performance high-carbon steel wire products have particular high requirements on cleanliness, segregation, decarburization, and surface quality. To obtain high-purity molten steel, high-homogenized cast billet and high-purity wire rod, on the basis of a conventional smelting process, during hot metal smelting, the S content in the molten steel is reduced to an extremely low level. In addition, high-quality scrap is used in the converter to minimize sulfur reversion, thereby comprehensively reducing desulfurization burden during the refining process. Refining desulfurization primarily relies on intensive bottom blowing and intense stirring to promote slag-metal reactions for desulfurization. However, this method is highly prone to causing slag entrapment or altering the type of inclusions through slag-metal reactions. Therefore, according to the present disclosure, the S content is reduced to a relatively low level during KR and converter stages, thereby avoiding intense slag-metal reactions. This prevents the formation of large-sized inclusions in the molten steel and facilitates the removal of the same. Cold-rolled silicon steel and titanium-free thick-plate scrap (such as pipeline steel and bridge steel) are selected for smelting. Meanwhile, a slide gate is used for slag retention in the converter, which can effectively avoid slag carry-over that leads to reversion of Al, Ti, P, and other elements, and the precipitation of brittle inclusions such as titanium oxide and titanium nitride during the continuous casting process is further prevented.

Secondly, in addition to using low-phosphorus and clean scrap to reduce the introduction of impurity elements during the converter smelting, lime and pellets are accurately added for slag formation at each stage of converter blowing, thereby maintaining a suitable basicity and oxidizability of the slag during the early, middle, and late stages of blowing and enhancing slag dephosphorization. In particular, dephosphorization in the early stage of converter blowing needs to be achieved. On the basis of the conventional dephosphorization process, bottom blowing is carried out in the early stage of converter blowing, and intensive bottom blowing stirring is conducted for a certain period of time to promote slag-metal reactions, thereby achieving effective dephosphorization control in the early stage. The middle stage of converter blowing is mainly focused on high-speed decarburization, during which the slag is prone to drying out. Therefore, it is necessary to accurately control addition amounts of the lime and pellets during the blowing to maintain the oxidizability and basicity of the slag in the middle stage, so that phosphorus reversion during the high-speed decarburization period can be significantly reduced. In the late stage of converter blowing, the slag with ultra-high basicity and high oxidizability is adopted to ensure high-temperature and low-phosphorus tapping in the late stage of the blowing, thereby obtaining low-phosphorus molten steel. In addition, the tapping temperature should meet the requirement for direct transfer to RH station for treatment. The problems such as nitrogen pickup and slag entrapment during the LF heating are avoided, and the cleanliness of the molten steel is improved.

Secondly, during converter smelting of the high-carbon steel wire, a low-carbon tapping process is adopted, and the oxidizability of the molten steel is appropriately increased to completely oxidize the small amounts of Al, Ti, and other elements introduced by the alloys, thereby removing the same the molten steel. In addition, prior to tapping, a small amount of carbon powder and metallic manganese are added in advance for pre-deoxidation to further reduce the oxidizability of the molten steel, thereby significantly decreasing the total content of silicon oxide, alumina, and the like formed during subsequent deoxidation and alloying. The adoption of incomplete deoxidation using carbon powder and metallic manganese can avoid excessive gas absorption by the molten steel and reduce N content in the molten steel. Combined with the use of asymmetric small-to-medium flow bottom blowing in the ladle, the formation of bias flow can be prevented, and the dissolution of carbon powder into the molten steel can be accelerated. Upon completion of tapping, silicon carbide is added to deoxidize and modify the slag. The slide gate for slag retention can control the amount of slag carry-over to a low level. After modification with silicon carbide, the oxidizability of the slag is controlled at a low level; and a medium-basicity silicate synthetic slag is added to cover the silicon carbide, thereby avoiding air burning loss and improving the deoxidation and modification effect of the slag. In addition, the synthetic slag in the form of calcium silicate compounds, benefiting from a low CaO content, can reduce the entrainment of CaO into the molten steel, thereby enabling the formation of deoxidation products dominated by SiO₂ and MnO components in the molten steel.

The semi-deoxidized molten steel is directly transported to the RH for treatment. The carbon in the molten steel is configured to reduce the oxygen content to a low level under high vacuum. In addition, the silicon carbide is added to enhance complex deoxidation with C and Si, reducing the total oxygen content in the molten steel to an extremely low level. Subsequently, a low-carbon carburizer, ultra-pure silicon, metallic manganese, ferrochrome, ferrovanadium, and other are added in sequence for alloying. The silicon carbide can increase C and Si contents of the molten steel, so that the required addition amount of carbon powder is reduced, and the temperature drop caused by the addition of large amount of carbon powder can be mitigated. Furthermore, the addition of SiC enables concurrent deoxidation by Si and C, so that the oxygen content can be reduced to an extremely low level. Heat released by slight oxidation of element Si can stabilize the temperature of the molten steel. Under high vacuum, the element carbon participates extensively in deoxidation, which also reduces the oxidation of other alloying elements such as Mn and Cr, thereby improving the yield of the alloying element. In addition, the total amount of oxide inclusions generated is reduced, the element Si lowers the final oxygen content of the molten steel. For a few high- carbon steels that may require the addition of a small amount of metallic aluminum, metallic aluminum can be added after the Si and C deoxidation in the vacuum furnace is completed, the aluminum oxidation can be significantly reduced, alumina- type inclusions can be reduced, and the cleanliness of the molten steel is improved.

Finally, the use of ladle refractory materials, vacuum furnace refractory materials, and continuous casting refractory materials (the "three main components") with low alumina content further reduces the sources of alumina inclusions. In addition, higher standards for refractory material quality decrease erosion of the refractory material and eliminate exogenous magnesia inclusions. Relevant research results show that high-melting-point exogenous inclusions such as alumina, magnesia, and magnesia-alumina spinel are the primary inclusions responsible for fatigue fracture in springs, brittle fracture during drawing of tire cord steel, and torsional brittle fracture in the cable steel. In an early stage of RH vacuum furnace process, deep vacuum and a medium-basicity slag system are employed to rapidly adsorb and remove acidic low-melting-point SiO₂-MnO inclusions. In the middle and late stages, a weak circulation stirring mode is adopted to avoid sustained high-intensity scouring of the refractories by the molten steel, allowing composite inclusions formed by minor refractory material erosion to float up and be removed. After vacuum breaking, asymmetric soft stirring and molten steel killing are further implemented to prevent slag entrapment caused by surface disturbance and to facilitate rapid flotation of remaining inclusions, thereby obtaining high-purity molten steel.

During continuous casting, high-basicity magnesium gunning mix is used to adsorb inclusions, and tundish electromagnetic induction heating, mold electromagnetic stirring and other technologies are used to further promote the floating and removal of inclusions.

During continuous casting, superheat casting is stabilized in a narrow range, and a proper superheat is adjusted according to C and Si contents of the molten steel. When the C content is low and the Si content is high, the superheat is appropriately increased to avoid a situation that is prone to cracking during reduction and straightening due to excessive hardness caused by low superheat. In addition, the appropriate increase of the superheat is beneficial to reduction. Combined with the control of an appropriate reduction amount, a segregation problem of the cast billet can be significantly improved. When the C content is high and the Si content is low, the superheat is moderately reduced, but it is still higher than that in the conventional process. Appropriate reduction process and cooling water flow rate are matched to ensure the proportion of a liquid phase region in each zone, and a gradual decrease mode of reduction is adopted to ensure the constant total reduction, weaken central segregation, and avoid internal cracks caused by excessive reduction. Controlling stable mold level fluctuation can completely avoid the problem of mold slag entrainment. The partial deoxidation process of converter tapping, RH vacuum degassing and other technologies, coupled with continuous casting cooling intensity control and constant speed casting technology, can reduce the generation of precipitates.

Finally, the reheating furnace adopts a technical concept of high-temperature heating and holding time prolonging to further promote uniform diffusion of alloying elements, thereby reducing the problems such as segregation and network carbide. In addition, a full grinding technology is adopted after cogging to eliminate surface quality problem of an original cast billet, and a high-temperature resistant coating is applied to the rolled billet to mitigate surface decarburization of the cast billet and improve microstructural homogeneity. Sorbite and pearlite microstructures are obtained by using a rolling-controlled and air-controlled technology, martensite and ferrite microstructures are reduced, and a high-purity high-carbon steel wire rod products is obtained for processing and preparing various high-carbon steel products.
(1) In the conventional process of smelting spring steel, a general desulfurization task is mainly in an LF refining station. The S content in the molten steel is controlled to an extremely low level during KR and converter stages, which effectively avoids slag entrapment and changes in inclusion types caused by extensive desulfurization during refining and can effectively reduce the size of inclusions while precisely controlling inclusion types.
(2) A double-slag efficient dephosphorization process has been developed for the converter. By designing the basicity and oxidizability of the slag, and bottom-blowing stirring in the early stage of blowing, low-phosphorus semi-steel molten steel is obtained in combination with molten steel temperature control. A technology for controlling the oxidizability of the slag during the high-speed decarburization period has been developed to avoid the problem of slag drying out and phosphorus reversion. Combined with the control technology for high-basicity and high-oxidizability slag in the late stage of the converter, high-temperature and low-phosphorus molten steel is achieved.
(3) Refectory materials for the ladle, RH vacuum furnace and continuous casting, as well as accessories, are all high-cleanliness standard materials, which can reduce an erosion problem caused by high-carbon and silicate inclusions and effectively control exogeneous inclusions, thereby providing an effective control method for exogeneous harmful inclusions in high-quality wire products.
(4) A full-process asymmetric flow rate control method for a dual-bottom-blowing ladle is innovatively proposed, which can effectively reduce a stirring dead zone of the molten steel caused by convection, significantly promote the flotation and removal of inclusions, and reduce gas consumption, providing positive significance for both improving molten steel quality and reducing costs.
(5) The full-process system design, which taking into account the control of various impurity elements and inclusions in the steel, can reduce the impurity element content and gas content in the steel. In addition, the size and quantity of both endogenous and exogenous inclusions can be greatly reduced, thereby remarkably improving the cleanliness of the molten steel.
(6) A semi-killed deoxidation process for converter tapping of high-carbon steel is precisely designed, which breaks away from conventional technological methods. Specifically, the converter tapping process is designed to first adopt partial deoxidation using a small amount of carbon powder and metallic manganese, combined with strong deoxidation and carburization using silicon carbide under RH vacuum conditions. This avoids gas pickup during the converter tapping deoxidation and alloying process and enables precise control of low- melting- point SiO₂- MnO- based inclusions. The combined C and Si deoxidation and variable vacuum intensity operation in the RH vacuum furnace not only reduce the number and size of inclusions but also control the types of low-melting-point plastic inclusions.

A used precise segmented reduction process, combined with high-temperature and long-term holding technology in the reheating furnace, can further promote uniform diffusion of elements. Moreover, high-temperature resistant coating technology is employed to effectively control the problem of surface decarburization of the cast billet, thereby comprehensively improving the quality of the cast billet.

The present disclosure primarily achieves reduced impurity element content in molten steel through systematic design of the smelting process and control standards for raw materials and auxiliary materials. By developing efficient deoxidation, alloying, and refining technologies, the high-purity molten steel is obtained, and plasticization and miniaturization of inclusions are achieved. Furthermore, a high-homogenized cast billet and a high-quality wire rod are obtained by using accurate continuous casting and rolling control technological methods, thereby providing a high-purity base material for a high-end wire product. The present disclosure provides a high-purity high-carbon steel wire and a production method therefor, which can be used for producing a high-cleanliness and high-homogenized wire rod product.

According to the present disclosure, deep desulfurization and converter double-slag dephosphorization technologies are employed. During converter tapping, part of carbon powder and part of metallic manganese are added to enable partial deoxidation and alloying, thereby controlling the oxygen content in molten steel, reducing Al and Ti contents, and reducing nitrogen pickup of the molten steel. Afterwards, a medium-basicity synthetic slag with a specific phase is added to enhance inclusion adsorption and control the types of the inclusions. The tapped molten steel directly enters the RH vacuum furnace without refining treatment. Deep vacuum degassing and inclusion removal are carried out at first. Subsequently, the circulation flow rate is reduced by reducing RH pumping cavity and increasing the gas flow rate, thereby mitigating erosion of the refractory materials, enhancing inclusion removal, and improving cleanliness. Combined with the control of physical and chemical indexes of tundish refractory materials, alloys and accessories, the exogeneous brittle inclusions are reduced. During continuous casting, the covering flux, the mold flux and the like are controlled to adsorb inclusions to improve cleanliness. During continuous casting, technologies such as accurate reduction based on the solid fraction is adopted to reduce segregation. Implementing high-temperature heating, billet protection, heating time prolonging, and the like can mitigate segregation and improve the quality of the wire rod.

### BRIEF DESCRIPTION OF THE DRAWINGS

FIG. 1 is a flowchart according to the present disclosure.

### DETAILED DESCRIPTION OF THE EMBODIMENTS

The present disclosure is further described below with reference to specific implementations. It should be understood that the following specific embodiments are only used to illustrate the present disclosure and are not used to limit the scope of the present disclosure.

With reference to FIG. 1, a method for manufacturing a high-purity high-carbon steel wire is carried out according to the following processes: hot metal pretreatment, converter smelting, RH vacuum treatment, bloom continuous casting, cogging and grinding, high-speed wire-rod rolling, Stelmor air cooling, and finished wire rod obtaining. Specifically including the following steps.

Step 1: Low-sulfur hot metal is obtained through KR hot metal pretreatment, and the low-sulfur hot metal is charged into a converter. Further, a KR arrival temperature is ≥1380°C, and in the hot metal, an S content is ≤0.045%, a C content is 4.1% to 4.6%, an Si content is 0.25% to 0.60%, a Ti content is ≤0.03%, a P content is ≤0.11%, with the balancing being Fe and other inevitable impurity elements. Upon arrival at a KR station, a blast furnace slag is skimmed off with a slag skimming rate of ≥95%; then, a desulfurizing agent is added for desulfurization, and after desulfurization, slag skimming is carried out again with a slag skimming rate of ≥95%; subsequently, the desulfurizing agent is added for the second desulfurization, with a slag skimming rate of ≥ 98%; and a KR departure temperature is controlled to be ≥1330°C, and a departure S content is controlled to be ≤0.0008%.

Step 2. Converter smelting is carried out with a converter charge of 145±5 t and a hot metal ratio of 80% to 90%, where clean scrap is selected for smelting, and the converter adopts a double-slag dephosphorization process. Intensive bottom-blowing stirring is adopted in an early stage of converter blowing, with a high lance position and a low oxygen flow rate, and a medium-basicity slag system with basicity of 1.8 to 2.2 is adopted; pellets are added to control a T.Fe content in the slag to be ≥25%; oxygen blowing is stopped upon completion of early-stage blowing, a temperature is controlled to be 1380°C to 1430°C; bottom-blowing stirring is carried out for more than 3 min until a P content is ≤0.016%, followed by slag removal; after the slag removal is completed, blowing is continued with a low lance position and a high oxygen supply flow rate; lime is added to form a high-basicity slag system, and pellets are to control a minimum T.Fe to be ≥15% during blowing; and at the end of blowing, the temperature is controlled to be ≥1650°C, the T.Fe content is controlled to be ≥25%, and the basicity is controlled to be ≥6; and slag removal is carried out at first, and upon completing the slag removal, tapping is carried out while retaining the slag with a slide gate.

Further, the clean scrap used by the converter includes composition as follows: less than or equal to 0.015% of P, less than or equal to 0.0050% of S, less than or equal to 0.01% of Ti, and conventional elements such as C, Si, Al, Mn, Fe; and at the end of converter blowing, a C content is 0.03% to 0.07%, an O content is 0.035% to 0.075%, a P content is ≤0.008%, and a tapping weight of the converter is 135±5 t.

Step 3. During converter tapping, at the start of tapping, 30% to 40% of low-nitrogen carburizer is added into a ladle at first, and 20% to 30% of metallic manganese is added for pre-deoxidation, tapping is completed after the added low-nitrogen carburizer and metallic manganese are fully dissolved into molten steel and no carbon powder particles float on the surface, and then silicon carbide and a synthetic slag are added into a ladle slag surface in sequence to deoxidize the slag surface and form slag. During converting tapping, ladle bottom blowing is maintained throughout the entire process, where in dual bottom blowing of the ladle, one porous plug has a maximum flow rate of 600 NL/min to 800 NL/min, and the other porous plug has a flow rate of 30% to 50% of the maximum flow rate, the two porous plugs are arranged on the bottom of the ladle at an angle of 135 degrees, located at a position 55% of a radius from the center of the ladle, and configured to blow argon into the molten steel to stir the molten steel and the slag.

A used ladle brick is a magnesia-carbon brick, which includes less than or equal to 3.0% of magnesium aluminate spinel, less than or equal to 3% of C, with the balance being inevitable impurity composition.

The low-carbon nitrogen carburizer added during converter tapping includes less than or equal to 0.045% of N, with the balance being C and inevitable impurity elements. The metallic manganese includes more than or equal to 99% of Mn, less than or equal to 0.003% of Ti, less than or equal to 0.005% of Al, less than or equal to 0.0065% of P, less than or equal to 0.0035% of S, with the balance being iron and inevitable impurity elements. The silicon carbide includes more than or equal to 98% of SiC, and other inevitable impurity elements. The synthetic slag includes composition as follows: 45% to 55% of CaO, 20% to 30% of SiO₂, 5% to 10% of CaF₂, 1% to 3% of MnO, less than or equal to 3% of MgO, less than or equal to 1.5% of Al₂O₃, and other inevitable impurity composition, and has a basicity of 1.5 to 2.0. In phase composition of the synthetic slag, monocalcium silicate accounts for 35% to 45%, dicalcium silicate accounts for 15% to 25%, and the others are CaO, CaF₂, MnO, and inevitable phases.

Upon completion of converter tapping, silicon carbide is added to deoxidize the ladle slag, with at an addition amount of 0.5 kg/t to 1.5 kg/t, and after the silicon carbide is added, a synthetic slag is added for slag formation, with an addition amount of 8 kg/t to 12 kg/t. Dual bottom blowing flow rates of the ladle are controlled at 150 NL/min to 250 NL/min after the synthetic slag is added, and the ladle is transported to RH for treatment after the synthetic slag is evenly spread.

Step 4: during RH furnace refining, a RH arrival temperature is controlled to be ≥1590°C, with a C content of ≥0.2%, an Mn content of 0.15-0.35%, and an oxygen content of ≤0.020%; during rapid evacuation treatment upon arrival at the RH station, an operating pressure of the vacuum chamber is controlled to be ≤1 mbar, and the lift gas flow rate is controlled to be 150 Nm³/min to 200 Nm³/min. Silicon carbide is added for deoxidation according to arrival composition, and deep vacuum treatment time is controlled to be ≥15 min, a sample is taken for composition test, and based on a composition test result and a composition requirement of a smelted steel grade, one or more of low-nitrogen carburizer, ultra-pure silicon, metallic manganese, ferrochrome, and ferrovanadium is selected for alloying. After the composition meets standards, a pumping capacity of a RH vacuum system is reduced by 40% to 60%, the lift gas flow rate is reduced to 80 Nm³/min to 100 Nm³/min, and the pressure in the vacuum chamber is increased to 50 mbar and more, and after carrying out net circulation for ≥5 min, vacuum is carried out.

A refractory material used for a dipping tube and a bottom tank of a RH vacuum furnace is an ultra-low-carbon magnesite-chrome brick, which includes less than or equal to 1.5% of C, 85% to 95% of MgO, 5% to 12% of Cr₂O₃, less than or equal to 3.0% of magnesium aluminate spinel, and other inevitable impurity composition.

The low-carbon nitrogen carburizer added during RH vacuum treatment includes less than or equal to 0.045% of N, with the balance being C and inevitable impurity elements. The metallic manganese includes more than or equal to 99% of Mn, less than or equal to 0.003% of Ti, less than or equal to 0.005% of Al, less than or equal to 0.0065% of P, less than or equal to 0.0035% of S, with the balance being iron and inevitable impurity elements. The silicon carbide includes more than or equal to 98% of SiC, and other inevitable impurity elements. The ultra-pure silicone includes 80% to 85% of Si, less than or equal to 0.0035% of Al, less than or equal to 0.001% of Ti, less than or equal to 0.005% of P, less than or equal to 0.0025% of S, with the balance being iron and inevitable impurity elements. The ferrochrome includes 55% to 60% of Cr, less than or equal to 1.8% of C, less than or equal to 0.006% of S, less than or equal to 0.013% of P, with the balance being iron and inevitable impurity elements. The ferrovanadium includes 45% to 50% of V, less than or equal to 1.6% of C, less than or equal to 0.005% of S, less than or equal to 0.012% of P, with the balance being iron and inevitable impurity elements.

After vacuum breaking in RH, soft stirring time is carried out for ≥6 min, the maximum flow rate of one of the dual porous plugs is controlled to be 60 NL/min to 80 NL/min, and the flow rate of the other porous plug is controlled to be 40% to 50% of the maximum flow rate; and the ladle is transported to a continuous casting platform to stand for 10 min and more, followed by casting.

S5. Bloom continuous casting is employed, where the bloom has a cross-section of 300 mm×390 mm, protective casting is implemented throughout the entire continuous casting process, a low-basicity and low-alumina tundish covering flux is used, and a superheat fluctuation of the molten steel in the tundish is controlled to be ≤5°C by using tundish electromagnetic induction heating equipment, where tundish induction heating is carried out with a current of 1500 A to 1800 A and a voltage of 1600 V to 2000 V; when a carbon content in the steel is 0.5%≤C<0.8%, a superheat of the molten steel is controlled to be 20°C to 35°C; and when a carbon content in the steel is that 0.8%≤C<1.0%, the superheat of the molten steel is controlled to be 30°C to 45°C, a tundish tonnage is maintained at 48±1 tons, and the tonnage during ladle change at 40 tons to 45 tons.

The mold electromagnetic stirring is carried out with a current of 450 A 650 A and a frequency of 6 Hz to 8 Hz, a mold water flow rate is set to 2750 NL/min to 3050 NL/min, a secondary cooling segment water flow rate is set to 550 NL/min to 650 NL/min, and a mold level fluctuation is set to ≤2 mm; continuous casting is carried out at a constant casting speed, and the continuous casting speed is controlled at 0.6 m/min to 0.7 m/min.

A solid fraction fs at the solidification center of a continuously cast billet is divided into four ranges, when 0.1≤fs<0.3, a reduction ratio accounts for 10% to 15%; when 0.3≤fs<0.5, a reduction ratio accounts for 20% to 30%; when 0.5≤fs<0.8, a reduction ratio accounts for 50% to 60%; when 0.8≤fs<1, a reduction ratio accounts for 10% to 20%; and a total reduction amount is controlled at 15 mm to 30 mm, thereby obtaining a cast billet with C segregation index of 0.95 to 1.05.

The low-basicity and low-alumina tundish covering flux for continuous casting includes main composition as follows: 40%-50% of CaO, 30% to 40% of /SiO₂, 3% to 6% of CaF₂, less than or equal to 2% of Al₂O₃, 3% to 6% of MgO, and other inevitable composition.

A magnesia spraying material for an inner wall of the tundish includes composition as follows: more than or equal to 80% of MgO, 5% to 10% of CaO, 1% to 3% of SiO₂, and other inevitable composition.

An overall submerged entry nozzle is used for casting, an insertion depth of the submerged entry nozzle is 10 mm to 15 mm, a mold flux has a slag layer thickness of 10 mm to 20 mm and a consumption rate of 0.15 kg/ton to 0.25 kg/ton.

Each of a stopper rod and the submerged entry nozzle is made of a magnesia carbon material, the stopper rod further includes the following composition in mass percentage: 80% to 85% of MgO, 8% to 12% of C, less than or equal to 1.5% of Al₂O₃, 1% to 4% of SiC, 2% to 3% of SiO₂, and other inevitable impurity composition.

The submerged entry nozzle has an inner wall thickness of 5 mm to 7 mm, and includes the following composition in mass percentage: 75% to 80% of MgO, 6% to 10% of C, 3% to 5% of SiC, 5% to 10% of SiO₂, and other inevitable impurity composition.

Step 6: During cogging and grinding, the continuously cast billet is heated in a cogging reheating furnace and undergoes soaking and heat preservation, a billet temperature is controlled to be 1100°C to 1200°C, and an initial rolling temperature is controlled to be 1040°C to 1180°C; a rolled billet is obtained after cogging and rolling; the rolled billet is subjected to magnetic particle inspection, followed by full surface grinding; and for a position with an apparent flaw detection defect on the surface, spot grinding is carried out additionally, with an average grinding depth of ≥0.5 mm.

During coating spraying of the rolled billet, a high-temperature-resistant coating is sprayed onto the surface of the ground rolled billet, with a thickness of 0.3 mm to 1.5 mm.

In a case of controlling an atmosphere in the reheating furnace, the rolled billet after coating spraying is heated in a steel-rolling reheating furnace and undergoes soaking and heat preservation, a temperature of the rolled billet in the steel-rolling reheating furnace is controlled at 1030°C to 1190°C, an initial rolling temperature is controlled at 910°C to 1170°C, a finish rolling entry temperature is controlled at 840°C to 960°C, and a finish rolling exit temperature is controlled at 990°C to 1050°C; and in percent by volume, a total content of H₂O and O₂ in atmosphere composition in the reheating furnace is ≤2.5%.

Step 7. During rolling and air cooling, a rolled wire obtained in a high-speed wire rod rolling procedure is subjected to temperature-controlled air cooling, and a wire laying temperature of an air cooling line is controlled at 820°C to 925°C.

A coating is sprayed for protection before the rolled billet enters the reheating furnace, where the coating has a thickness of 0.3 mm to 1.5 mm, and the high-temperature coating includes CaO, SiO₂, Al₂O₃, MgO, ZrO, C, as well as small amounts of alkali metal oxides, inorganic binders, and surfactants.

Further, the bloom is cogged into a billet with a cross-section of 140 mm×140 mm, followed by flow inspection and grinding, heating in a reheating furnace, rolling, and controlled cooling on a Stelmor air-cooling line, so that an obtained wire rod is free from surface defects such as seams, scabs, and scratches, and there is no fully decarburized layer on a surface thereof.

### Embodiment

A generated high-purity high-carbon steel wire, in addition to alloying elements and Fe element, includes the following chemical composition in mass percentage: 0.5% to 1.0% of C, less than or equal to 0.008% of P, less than or equal to 0.0025% of S, less than or equal to 0.0010% of T.O, less than or equal to 0.0020% of N, less than or equal to 0.0002% of H, less than or equal to 0.0010% of Alt, and less than or equal to 0.0005% of Ti.

The technical production process of the present disclosure is introduced with spring steel 55SiCr/65Mn, cord steel 72A/82A/97A and cable steel 87B/92Si as examples.

Spring steel 55SiCr includes the following chemical composition in mass percentage: 0.50% to 0.60% of C, 1.35% to 1.65% of Si, 0.60% to 0.80% of Mn, 0.55% to 0.80% of Cr, and 0.15% to 0.35% of V

Spring steel 65Mn includes the following chemical composition in mass percentage: 0.60% to 0.70% of C, 0.20% to 0.40% of Si, and 0.90% to 1.00% of Mn.

Cord wire 72A includes the following chemical composition in mass percentage: 0.70% to 0.78% of C, 0.15% to 0.30% of Si, and 0.50% to 0.60% of Mn.

Cord wire 82A includes the following chemical composition in mass percentage: 0.78% to 0.86% of C, 0.15% to 0.35% of Si, and 0.50% to 0.65% of Mn.

Cord wire 97A includes the following chemical composition in mass percentage: 0.95% to 1.00% of C, 0.15% to 0.30% of Si, and 0.35% to 0.45% of Mn.

Cable steel 87B includes the following chemical composition in mass percentage: 0.85% to 0.90% of C, 0.45% to 0.60% of Si, 0.70% to 0.85% of Mn, 0.20% to 0.35% of Cr, and 0.02% to 0.05% of V.

Cable steel 92Si includes the following chemical composition in mass percentage: 0.90% to 0.95% of C, 1.1% to 1.3% of Si, 0.75% to 0.90% of Mn, 0.20% to 0.35% of Cr, and 0.01% to 0.04% of V.

The high-purity high-carbon steel wire is produced according to the following technological processes: hot metal pretreatment, converter smelting, RH vacuum treatment, bloom continuous casting, cogging and grinding, high-speed wire-rod rolling, Stelmor air cooling, and finished wire rod obtaining.

### Step 1: KR hot metal pretreatment

The hot metal is transported to a KR treatment station and undergoes three times of slag skimming and twice deep desulfurization to obtain low-sulfur hot metal, and then the hot metal is charged into a converter for smelting.

**Table 1 Main parameters of hot metal arriving at KR station for spring steel**

| Steel grade | Parameter | Arrival temperature , °C | S content, % | C content, % | Si content, % | Ti content, % | P content, % |
|---|---|---|---|---|---|---|---|
| 55SiC r | Embodimen t 1 | 1390 | 0.26 | 4.2 | 0.55 | 0.013 | 0.092 |
| | Embodimen t 2 | 1446 | 0.32 | 4.1 | 0.33 | 0.018 | 0.085 |
| | Embodimen t 3 | 1435 | 0.45 | 4.4 | 0.25 | 0.021 | 0.106 |
| 65Mn | Embodimen t 4 | 1380 | 0.20 | 4.6 | 0.60 | 0.030 | 0.110 |
| | Embodimen t 5 | 1453 | 0.19 | 4.2 | 0.37 | 0.025 | 0.102 |
| | Embodimen t 6 | 1433 | 0.33 | 4.3 | 0.31 | 0.019 | 0.093 |

**Table 2 Main parameters for KR desulfurization treatment for spring steel**

| Steel grade | Parameter | First slag skimming rate, % | Second slag skimming rate, % | Third slag skimming rate, % | Departure temperature, °C | S content, % |
|---|---|---|---|---|---|---|
| 55SiCr | Embodiment 1 | 96 | 97 | 98 | 1354 | 0.0005 |
| | Embodiment 2 | 95 | 96 | 99 | 1401 | 0.0003 |
| | Embodiment 3 | 97 | 95 | 98 | 1397 | 0.0006 |
| 65Mn | Embodiment 4 | 98 | 97 | 98 | 1330 | 0.0008 |
| | Embodiment 5 | 95 | 98 | 99 | 1411 | 0.0005 |
| | Embodiment 6 | 97 | 96 | 98 | 1402 | 0.0004 |

**Table 3 Main parameters of hot metal arriving at KR station for cord steel**

| Steel grad e | Parameter | Arrival temperature , °C | S content, % | C content, % | Si content, % | Ti content, % | P content, % |
|---|---|---|---|---|---|---|---|
| 72A | Embodimen t 7 | 1389 | 0.33 | 4.6 | 0.33 | 0.019 | 0.101 |
| | Embodimen t 8 | 1380 | 0.17 | 4.3 | 0.42 | 0.022 | 0.110 |
| | Embodimen t 9 | 1421 | 0.45 | 4.1 | 0.38 | 0.030 | 0.096 |
| 82A | Embodimen t 10 | 1395 | 0.28 | 4.3 | 0.53 | 0.021 | 0.095 |
| | Embodimen t 11 | 1437 | 0.22 | 4.2 | 0.60 | 0.028 | 0.086 |
| | Embodimen t 12 | 1455 | 0.36 | 4.5 | 0.25 | 0.016 | 0.103 |
| 97A | Embodimen t 13 | 1393 | 0.21 | 4.6 | 0.50 | 0.024 | 0.088 |
| | Embodimen t 14 | 1416 | 0.18 | 4.4 | 0.36 | 0.020 | 0.107 |
| | Embodimen t 15 | 1383 | 0.39 | 4.3 | 0.29 | 0.017 | 0.095 |

**Table 4 Main parameters for KR desulfurization treatment for cord steel**

| Steel grade | Parameter | First slag skimming rate, % | Second slag skimming rate, % | Third slag skimming rate, % | Departure temperature, °C | S content, % |
|---|---|---|---|---|---|---|
| 72A | Embodiment 7 | 95 | 98 | 99 | 1342 | 0.0008 |
| | Embodiment 8 | 97 | 96 | 98 | 1333 | 0.0005 |
| | Embodiment 9 | 98 | 95 | 98 | 1387 | 0.0004 |
| 8A | Embodiment 10 | 96 | 96 | 98 | 1340 | 0.0006 |
| | Embodiment 11 | 95 | 98 | 99 | 1396 | 0.0005 |
| | Embodiment 12 | 96 | 97 | 98 | 1408 | 0.0004 |
| 97 | Embodiment 13 | 95 | 98 | 99 | 1351 | 0.0007 |
| | Embodiment 14 | 97 | 96 | 99 | 1375 | 0.0006 |
| | Embodiment 15 | 98 | 95 | 98 | 1330 | 0.0003 |

**Table 5 Main parameters of hot metal arriving at KR station for cable steel**

| Steel grad e | Parameter | KR Arrival temperature , °C | S content, % | C content, % | Si content, % | Ti content, % | P content, % |
|---|---|---|---|---|---|---|---|
| 87B | Embodimen t 16 | 1382 | 0.34 | 4.3 | 0.23 | 0.015 | 0.097 |
| | Embodimen t 17 | 1410 | 0.29 | 4.1 | 0.28 | 0.030 | 0.088 |
| | Embodimen t 18 | 1397 | 0.36 | 4.4 | 0.55 | 0.016 | 0.110 |
| 92Si | Embodimen t 19 | 1428 | 0.45 | 4.6 | 0.60 | 0.022 | 0.083 |
| | Embodimen t 20 | 1403 | 0.19 | 4.2 | 0.36 | 0.018 | 0.103 |
| | Embodimen t 21 | 1390 | 0.27 | 4.3 | 0.31 | 0.021 | 0.100 |

**Table 6 Main parameters for KR desulfurization treatment of cable steel**

| Steel grade | Parameter | First slag skimming rate, % | Second slag skimming rate, % | Third slag skimming rate, % | Departure temperature, °C | S content, % |
|---|---|---|---|---|---|---|
| 87B | Embodiment 16 | 97 | 97 | 99 | 1330 | 0.0004 |
| | Embodiment 17 | 96 | 95 | 98 | 1368 | 0.0006 |
| | Embodiment 18 | 96 | 98 | 98 | 1351 | 0.0005 |
| 92Si | Embodiment 19 | 95 | 95 | 99 | 1389 | 0.0004 |
| | Embodiment 20 | 96 | 96 | 99 | 1357 | 0.0007 |
| | Embodiment 21 | 97 | 96 | 98 | 1342 | 0.0006 |

### Step 2: Converter smelting

After the hot metal and clean scrap are charged into the converter, double-slag dephosphorization is employed. Intensive bottom-blowing stirring is employed in an early stage of converter blowing, with a high lance position and a low oxygen flow rate, a medium-basicity and high-oxidizing slag system is adopted. Upon completion of the early-stage blowing, bottom-blowing stirring is carried out, followed by slag removal. After slag removal is completed, blowing is continued with a low lance position and a high oxygen supply flow rate. Lime is added to form a high-basicity and high-oxidizing slag system, and a T.Fe content during blowing is controlled. At the end of blowing, slagging removal is carried out at first, and upon completing the slag removal, tapping is carried out using a slide gate for slag retention. The clean scrap used by the converter includes composition as follows: less than or equal to 0.015% of P, less than or equal to 0.0050% of S, less than or equal to 0.01% of Ti, and conventional C, Si, Al, Mn and Fe elements.

**Table 7 Main parameters of first stage of converter smelting for spring steel**

| Steel grade | Parameter | Convert er charge, t | Hot metal ratio, % | Slag basicit y at blow-off | T.Fe in slag at blow-off, % | Blow-off temperatu re, °C | Bottom-blow ing stirring time, min | P content, % |
|---|---|---|---|---|---|---|---|---|
| 55Si Cr | Embodim ent 1 | 140 | 90 | 2.2 | 28 | 1430 | 4.5 | 0.0133 |
| | Embodim ent 2 | 145 | 85 | 2.0 | 29 | 1422 | 3.0 | 0.0160 |
| | Embodim ent 3 | 143 | 88 | 1.9 | 25 | 1380 | 3.5 | 0.0155 |
| 65M n | Embodim ent 4 | 150 | 80 | 2.1 | 31 | 1396 | 5.0 | 0.0127 |
| | Embodim ent 5 | 148 | 86 | 1.8 | 27 | 1388 | 4.0 | 0.0151 |
| | Embodim ent 6 | 146 | 87 | 2.0 | 33 | 1415 | 5.5 | 0.0146 |

**Table 8 Main parameters of second stage of converter smelting for spring steel**

| Steel grad e | Paramete r | Conver ter charge, t | Lowe st T.Fe, % | Slag basicit y at blow-off | T.Fe in slag at blow-off , % | Blow-off temperat ure, °C | C in tapping ,% | O in tapping ,% | P in tapping ,% |
|---|---|---|---|---|---|---|---|---|---|
| 55Si Cr | Embodi ment 1 | 130 | 16 | 8 | 27 | 1665 | 0.045 | 0.051 | 0.0072 |
| | Embodi ment 2 | 136 | 18 | 9 | 30 | 1650 | 0.070 | 0.035 | 0.0043 |
| | Embodi ment 3 | 134 | 15 | 6 | 29 | 1672 | 0.035 | 0.075 | 0.0036 |
| 65M n | Embodi ment 4 | 140 | 23 | 7 | 28 | 1663 | 0.052 | 0.063 | 0.0065 |
| | Embodiment 5 | 136 | 21 | 11 | 25 | 1668 | 0.058 | 0.056 | 0.0080 |
| | Embodi ment 6 | 135 | 19 | 10 | 31 | 1657 | 0.065 | 0.047 | 0.0056 |

**Table 9 Main parameters of first stage of converter smelting for cord steel**

| Steel grade | Parameter | Converter charge, t | Hot metal ratio, % | Slag basicity at blow-off | T.Fe in slag at blow-off | Blow-off temperature , °C | Bottom-blowing stirring time, min | P content, % |
|---|---|---|---|---|---|---|---|---|
| 72A | Embodiment 7 | 145 | 86 | 1.8 | 26 | 1415 | 3.5 | 0.0149 |
| | Embodiment 8 | 144 | 88 | 2.2 | 28 | 1420 | 3.5 | 0.0153 |
| | Embodiment 9 | 146 | 86 | 1.8 | 30 | 1396 | 4.5 | 0.0136 |
| 82A | Embodiment 10 | 148 | 90 | 2.0 | 25 | 1400 | 4.0 | 0.0124 |
| | Embodiment 11 | 147 | 86 | 1.9 | 31 | 1380 | 5.0 | 0.0161 |
| | Embodiment 12 | 150 | 87 | 2.1 | 26 | 1419 | 3.5 | 0.0156 |
| 97A | Embodiment 13 | 143 | 85 | 2.0 | 28 | 1407 | 4.5 | 0.0133 |
| | Embodiment 14 | 140 | 87 | 1.8 | 25 | 1389 | 3.0 | 0.0142 |
| | Embodiment 15 | 146 | 84 | 1.9 | 27 | 1396 | 3.5 | 0.0118 |

**Table 10 Main parameters of second stage of converter smelting for cord steel**

| Steel grade | Parameter | Converter charge, t | Lowest T.Fe, % | Slag basicity at blow-off | T.Fe in slag at blow-off , % | Blow-off temperature , °C | C in tapping ,% | O in tapping ,% | P in tapping ,% |
|---|---|---|---|---|---|---|---|---|---|
| 72 A | Embodiment 7 | 133 | 18 | 7 | 26 | 1655 | 0.056 | 0.046 | 0.0065 |
| | Embodiment 8 | 135 | 22 | 8 | 31 | 1658 | 0.045 | 0.058 | 0.0052 |
| | Embodiment 9 | 134 | 17 | 8 | 28 | 1662 | 0.038 | 0.070 | 0.0046 |
| 82 A | Embodiment 10 | 137 | 20 | 6 | 27 | 1673 | 0.063 | 0.035 | 0.0035 |
| | Embodiment 11 | 136 | 15 | 9 | 29 | 1669 | 0.070 | 0.037 | 0.0073 |
| | Embodiment 12 | 140 | 19 | 11 | 25 | 1670 | 0.035 | 0.070 | 0.0056 |
| 97 A | Embodiment 13 | 132 | 17 | 9 | 33 | 1663 | 0.044 | 0.063 | 0.0080 |
| | Embodiment 14 | 130 | 25 | 10 | 30 | 1650 | 0.050 | 0.055 | 0.0067 |
| | Embodiment 15 | 135 | 20 | 8 | 26 | 1667 | 0.061 | 0.049 | 0.0051 |

**Table 11 Main parameters of first stage of converter smelting for cable steel**

| Steel grade | Parameter | Converter charge, t | Hot metal ratio, % | Slag basicity at blow-off | T.Fe in slag at blow-off | Blow-off temperature , °C | Bottom-blowing stirring time, min | P content, % |
|---|---|---|---|---|---|---|---|---|
| 87B | Embodiment 16 | 142 | 88 | 2.0 | 25 | 1425 | 3.5 | 0.0145 |
| | Embodiment 17 | 148 | 83 | 2.1 | 26 | 1412 | 4.0 | 0.0153 |
| | Embodiment 18 | 150 | 90 | 1.8 | 27 | 1398 | 4.5 | 0.0160 |
| 92Si | Embodiment 19 | 140 | 85 | 1.9 | 32 | 1380 | 4.0 | 0.0138 |
| | Embodiment 20 | 144 | 80 | 1.9 | 28 | 1406 | 5.0 | 0.0121 |
| | Embodiment 21 | 146 | 86 | 2.2 | 26 | 1380 | 4.5 | 0.0136 |

**Table 12 Main parameters of second stage of converter smelting for cable steel**

| Steel grade | Parameter | Converter charge, t | Lowest T.Fe, % | Slag basicity at blow-off | T.Fe in slag at blow-off ,% | Blow-off temperature , °C | C in tapping ,% | O in tapping ,% | P in tapping ,% |
|---|---|---|---|---|---|---|---|---|---|
| 87B | Embodiment 16 | 131 | 19 | 6 | 26 | 1650 | 0.035 | 0.075 | 0.0056 |
| | Embodiment 17 | 136 | 15 | 7 | 29 | 1667 | 0.063 | 0.053 | 0.0061 |
| | Embodiment 18 | 140 | 18 | 9 | 25 | 1650 | 0.047 | 0.062 | 0.0047 |
| 92Si | Embodiment 19 | 130 | 21 | 10 | 27 | 1653 | 0.070 | 0.035 | 0.0035 |
| | Embodiment 20 | 135 | 20 | 8 | 28 | 1671 | 0.056 | 0.051 | 0.0072 |
| | Embodiment 21 | 137 | 17 | 7 | 31 | 1663 | 0.051 | 0.065 | 0.0080 |

### Step 3: Converter tapping

At the start of tapping, part of low-nitrogen carburizer and metallic manganese are added into to a ladle at first for pre-deoxidation, and tapping is completed after the added low-nitrogen carburizer and metallic manganese are fully dissolved into molten steel and no carbon powder particles float on the surface. Then silicon carbide and a synthetic slag are added to ladle slag surface in sequence to deoxidize the slag surface and form slag. During converting tapping, ladle bottom blowing is maintained throughout the entire process, where in dual bottom blowing of the ladle, one porous plug has a maximum flow rate of 600 NL/min to 800 NL/min, and the other porous plug has a flow rate of 30% to 50% of the maximum flow rate, the two porous plugs are arranged on the bottom of the ladle at an angle of 135 degrees, located at a position 55% of a radius from the center of the ladle, and configured to blow argon into the molten steel to stir the molten steel and the slag. A used ladle brick is a magnesia-carbon brick, which includes less than or equal to 3.0% of magnesium aluminate spinel, less than or equal to 3% of C, with the balance being inevitable impurity composition. The low-carbon nitrogen carburizer added during converter tapping includes less than or equal to 0.045% of N, with the balance being C and inevitable impurity elements. The metallic manganese includes more than or equal to 99% of Mn, less than or equal to 0.003% of Ti, less than or equal to 0.005% of Al, less than or equal to 0.0065% of P, less than or equal to 0.0035% of S, with the balance being iron and inevitable impurity elements. The silicon carbide includes more than or equal to 98% of SiC, and other inevitable impurity elements. The synthetic slag includes composition as follows: 45% to 55% of CaO, 20% to 30% of SiO₂, 5% to 10% of CaF₂, 1% to 3% of MnO, less than or equal to 3% of MgO, less than or equal to 1.5% of Al₂O₃, and other inevitable impurity composition, and has a basicity of 1.5 to 2.0. In phase composition of the synthetic slag, monocalcium silicate accounts for 35% to 45%, dicalcium silicate accounts for 15% to 25%, and the others are CaO, CaF₂, MnO, and inevitable phases.

Upon completion of converter tapping, silicon carbide is added to deoxidize the ladle slag, and after the silicon carbide is added, a synthetic slag is added for slag formation. The ladle flow rate is lowered after the synthetic slag is added, making dual bottom blowing flow rates consistent. The ladle is transported to RH for treatment after the synthetic slag is evenly spread.

**Table 13 Main Parameters of converter tapping for spring steel**

| Steel grade | Parameter | Maximum bottom blowing flow rate, NL/min | Small bottom blowing ratio, % | Addition amount of silicon carbide, kg/t | Synthetic slag basicity | Addition amount, kg/t | Bottom blowing in late stage, NL/min |
|---|---|---|---|---|---|---|---|
| 55SiCr | Embodiment 1 | 600 | 50 | 1.0 | 1.7 | 10 | 180 |
| | Embodiment 2 | 800 | 30 | 0.5 | 1.5 | 8 | 200 |
| | Embodiment 3 | 650 | 45 | 1.5 | 2.0 | 12 | 150 |
| 65Mn | Embodiment 4 | 700 | 40 | 1.4 | 1.9 | 11 | 250 |
| | Embodiment 5 | 750 | 35 | 1.3 | 1.8 | 10 | 190 |
| | Embodiment 6 | 700 | 40 | 0.8 | 1.6 | 9 | 210 |

**Table 14 Main Parameters of converter tapping for cord steel**

| Steel grade | Parameter | Maximum bottom blowing flow rate, NL/min | Small bottom blowing ratio, % | Addition amount of silicon carbide, kg/t | Synthetic slag basicity | Addition amount, kg/t | Bottom blowing in late stage, NL/min |
|---|---|---|---|---|---|---|---|
| 72A | Embodiment 7 | 700 | 40 | 0.9 | 1.6 | 9 | 190 |
| | Embodiment 8 | 750 | 45 | 1.1 | 1.7 | 9 | 220 |
| | Embodiment 9 | 600 | 50 | 1.5 | 2.0 | 11 | 180 |
| 82A | Embodiment 10 | 800 | 30 | 0.5 | 1.5 | 10 | 200 |
| | Embodiment 11 | 750 | 45 | 0.6 | 1.6 | 9 | 250 |
| | Embodiment 12 | 700 | 40 | 1.5 | 1.9 | 12 | 150 |
| 97A | Embodiment 13 | 600 | 45 | 1.4 | 1.8 | 8 | 200 |
| | Embodiment 14 | 800 | 45 | 1.3 | 1.7 | 9 | 250 |
| | Embodiment 15 | 750 | 35 | 1.2 | 1.8 | 11 | 190 |

**Table 15 Main Parameters of converter tapping for cable steel**

| Steel grade | Parameter | Maximum bottom blowing flow rate, NL/min | Small bottom blowing ratio, % | Addition amount of silicon carbide, kg/t | Synthetic slag basicity | Addition amount, kg/t | Bottom blowing in late stage, NL/min |
|---|---|---|---|---|---|---|---|
| 87B | Embodiment 16 | 700 | 40 | 1.5 | 2.0 | 11 | 200 |
| | Embodiment 17 | 600 | 45 | 0.9 | 1.8 | 8 | 250 |
| | Embodiment 18 | 750 | 35 | 1.3 | 1.7 | 11 | 190 |
| 92Si | Embodiment 19 | 800 | 40 | 0.5 | 1.9 | 9 | 150 |
| | Embodiment 20 | 650 | 50 | 1.2 | 1.6 | 10 | 220 |
| | Embodiment 21 | 750 | 40 | 1.4 | 1.8 | 12 | 180 |

### Step 4: RH furnace refining

Upon arrival at a KR station, rapid vacuum evacuation is carried, a high lift gas flow rate is set, followed by the addition of silicon carbide for deoxidation based on the arrival composition. Deep vacuum treatment is maintained for a specific duration, and a sample is taken for composition analysis. Based on a composition test result and a composition requirement of a smelted steel grade, one or more of low-nitrogen carburizer, ultra-pure silicon, metallic manganese, ferrochrome, and ferrovanadium is selected for alloying. After the composition meets standards, pumping capacity of a RH vacuum system is reduced, the lift gas flow rate is reduced, and the pressure in the vacuum chamber is increased. After carrying out net circulation for ≥5 min, vacuum breaking is carried out.

A refractory material used for a dipping tube and a bottom tank of a RH vacuum furnace is an ultra-low-carbon magnesite-chrome brick, which includes less than or equal to 1.5% of C, 85% to 95% of MgO, 5% to 12% of Cr₂O₃, less than or equal to 3.0% of magnesium aluminate spinel, and other inevitable impurity composition.

The low-carbon nitrogen carburizer added during RH vacuum treatment includes less than or equal to 0.045% of N, with the balance being C and inevitable impurity elements. The metallic manganese includes more than or equal to 99% of Mn, less than or equal to 0.003% of Ti, less than or equal to 0.005% of Al, less than or equal to 0.0065% of P, less than or equal to 0.0035% of S, with the balance being iron and inevitable impurity elements. The silicon carbide includes more than or equal to 98% of SiC, and other inevitable impurity elements. The ultra-pure silicone includes 80% to 85% of Si, less than or equal to 0.0035% of Al, less than or equal to 0.001% of Ti, less than or equal to 0.005% of P, less than or equal to 0.0025% of S, with the balance being iron and inevitable impurity elements. The ferrochrome includes 55% to 60% of Cr, less than or equal to 1.8% of C, less than or equal to 0.006% of S, less than or equal to 0.013% of P, with the balance being iron and inevitable impurity elements.

After vacuum breaking in RH, soft stirring time is carried out, the bottom blowing flow rates of the two porous plugs are set differently, where a smaller bottom blowing rate is 40% to 50% of the large bottom blowing flow rate. The ladle is transported to a continuous casting platform to stand for 10 min and more, followed by casting.

**Table 16 Parameters of RH arrival and deep vacuum treatment for spring steel**

| Steel grade | Parameter | Arrival Temperature , °C | C, % | Mn, % | O, % | Lowest pressure , mbar | Lift gas, Nm³/min | Treatment time, min |
|---|---|---|---|---|---|---|---|---|
| 55SiC r | Embodiment 1 | 1608 | 0.26 | 0.19 | 0.0157 | 0.5 | 150 | 18 |
| | Embodiment 2 | 1603 | 0.28 | 0.15 | 0.0132 | 1.0 | 200 | 15 |
| | Embodiment 3 | 1606 | 0.20 | 0.26 | 0.0200 | 0.8 | 180 | 16 |
| 65Mn | Embodiment 4 | 1598 | 0.25 | 0.23 | 0.0086 | 0.4 | 190 | 17 |
| | Embodiment 5 | 1597 | 0.27 | 0.28 | 0.0105 | 0.6 | 200 | 19 |
| | Embodiment 6 | 1590 | 0.31 | 0.35 | 0.0078 | 0.7 | 160 | 20 |

**Table 17 Parameters of late RH treatment stage and tapping for spring steel**

| Steel grade | Parameter | Decrease in pumping capacity, % | Lift gas, Nm³/min | Pressure , mbar | Net circulation , min | Soft stirring , min | Maximum bottom-blowing flow rate, NL/min | Flow rate ratio, % |
|---|---|---|---|---|---|---|---|---|
| 55Si Cr | Embodiment 1 | 40 | 90 | 90 | 6 | 8 | 80 | 50 |
| | Embodiment 2 | 60 | 80 | 78 | 7 | 7 | 70 | 45 |
| | Embodiment 3 | 50 | 100 | 50 | 8 | 6 | 60 | 50 |
| 65Mn | Embodiment 4 | 45 | 95 | 65 | 5 | 10 | 75 | 45 |
| | Embodiment 5 | 55 | 85 | 106 | 9 | 8 | 65 | 50 |
| | Embodiment 6 | 50 | 100 | 97 | 10 | 6 | 80 | 40 |

**Table 18 Parameters of RH arrival and deep vacuum treatment for cord steel**

| Steel grade | Parameter | Arrival Temperature, °C | C, % | Mn, % | O, % | Lowest pressure, mbar | Lift gas, Nm³/min | Treatment time, min |
|---|---|---|---|---|---|---|---|---|
| 72A | Embodiment 7 | 1615 | 0.20 | 0.15 | 0.0175 | 0.4 | 180 | 16 |
| | Embodiment 8 | 1618 | 0.23 | 0.23 | 0.0200 | 0.8 | 190 | 17 |
| | Embodiment 9 | 1612 | 0.25 | 0.27 | 0.0146 | 0.7 | 170 | 18 |
| 82A | Embodiment 10 | 1598 | 0.28 | 0.23 | 0.0086 | 1.0 | 150 | 15 |
| | Embodiment 11 | 1605 | 0.27 | 0.16 | 0.0128 | 0.7 | 160 | 18 |
| | Embodiment 12 | 1608 | 0.26 | 0.19 | 0.0159 | 0.5 | 200 | 19 |
| 97A | Embodiment 13 | 1590 | 0.34 | 0.15 | 0.0180 | 0.6 | 170 | 20 |
| | Embodiment 14 | 1595 | 0.31 | 0.19 | 0.0079 | 0.4 | 150 | 18 |
| | Embodiment 15 | 1596 | 0.29 | 0.18 | 0.0095 | 0.9 | 180 | 16 |

**Table 19 Parameters of late RH treatment stage and tapping for cord steel**

| Steel grade | Parameter | Decrease in pumping capacity, % | Lift gas, Nm³/min | Pressure , mbar | Net circulation , min | Soft stirring , min | Maximum bottom-blowing flow rate, NL/min | Flow rate ratio, % |
|---|---|---|---|---|---|---|---|---|
| 72A | Embodiment 7 | 45 | 100 | 110 | 10 | 10 | 80 | 50 |
| | Embodiment 8 | 55 | 90 | 88 | 5 | 8 | 70 | 45 |
| | Embodiment 9 | 50 | 80 | 50 | 8 | 6 | 75 | 45 |
| 82A | Embodiment 10 | 40 | 95 | 95 | 9 | 8 | 65 | 40 |
| | Embodiment 11 | 60 | 100 | 108 | 8 | 7 | 60 | 45 |
| | Embodiment 12 | 50 | 90 | 58 | 10 | 6 | 70 | 50 |
| 97A | Embodiment 13 | 40 | 95 | 79 | 7 | 8 | 80 | 45 |
| | Embodiment 14 | 60 | 88 | 72 | 6 | 7 | 75 | 45 |
| | Embodiment 15 | 50 | 96 | 66 | 7 | 6 | 65 | 40 |

**Table 20 Parameters of RH arrival and deep vacuum treatment for cable steel**

| Steel grade | Parameter | Arrival Temperature, °C | C, % | Mn, % | O, % | Lowest pressure, mbar | Lift gas, Nm³/min | Treatment time, min |
|---|---|---|---|---|---|---|---|---|
| 87B | Embodiment 16 | 1595 | 0.28 | 0.22 | 0.0153 | 0.5 | 180 | 16 |
| | Embodiment 17 | 1603 | 0.33 | 0.15 | 0.0092 | 0.4 | 160 | 19 |
| | Embodiment 18 | 1606 | 0.25 | 0.21 | 0.0109 | 1.0 | 150 | 20 |
| 92Si | Embodiment 19 | 1597 | 0.29 | 0.18 | 0.0096 | 0.3 | 190 | 17 |
| | Embodiment 20 | 1590 | 0.35 | 0.26 | 0.0083 | 0.4 | 170 | 15 |
| | Embodiment 21 | 1595 | 0.38 | 0.23 | 0.0075 | 0.6 | 180 | 16 |

**Table 21 Parameters of late RH treatment stage and tapping for cable steel**

| Steel grade | Parameter | Decrease in pumping capacity, % | Lift gas, Nm³/min | Pressure , mbar | Net circulation , min | Soft stirring , min | Maximum bottom-blowing flow rate, NL/min | Flow rate ratio, % |
|---|---|---|---|---|---|---|---|---|
| 87B | Embodiment 16 | 50 | 100 | 50 | 5 | 10 | 60 | 50 |
| | Embodiment 17 | 55 | 80 | 100 | 7 | 8 | 65 | 45 |
| | Embodiment 18 | 40 | 95 | 65 | 8 | 6 | 75 | 40 |
| 92Si | Embodiment 19 | 50 | 100 | 86 | 10 | 6 | 70 | 45 |
| | Embodiment 20 | 55 | 85 | 76 | 8 | 7 | 80 | 40 |
| | Embodiment 21 | 45 | 98 | 58 | 9 | 6 | 65 | 45 |

### Step 5: Bloom continuous casting

The bloom has a cross-section of 300 mm×390 mm, protective casting is implemented throughout the entire continuous casting process, a low-basicity and low-alumina tundish covering flux is used, and a superheat fluctuation of the molten steel in the tundish is controlled by using tundish electromagnetic induction heating equipment, where a current and voltage for tundish induction heating are set. The superheat of the molten steel in the tundish is adjusted according to the C and sulfur change of the steel grade, and the tundish tonnage is maintained stable during the casting and ladle change processes.

A current and a frequency for mold electromagnetic stirring are set, stirring is enhanced, the mold water flow rate and the secondary cooling segment water flow rate are set. Continuous casting is carried out at a constant casting speed, and a liquid level of the mold is maintained stable.

A solid fraction fs at the solidification center of a continuously cast billet is divided into four ranges, with different reduction amounts allocated to each range. When 0.1≤fs<0.3, a reduction ratio accounts for 10% to 15%; when 0.3≤fs<0.5, a reduction ratio accounts for 20% to 30%; when 0.5≤fs<0.8, a reduction ratio accounts for 50% to 60%; when 0.8≤fs<1, a reduction ratio accounts for 10% to 20%. A cast billet with C segregation index of 0.95 to 1.05 is obtained by controlling the reduction amount.

The low-basicity and low-alumina tundish covering flux for continuous casting includes main composition as follows: 40%-50% of CaO, 30% to 40% of /SiO₂, 3% to 6% of CaF₂, less than or equal to 2% of Al₂O₃, 3% to 6% of MgO, and other inevitable composition. A magnesia spraying material for an inner wall of the tundish includes composition as follows: more than or equal to 80% of MgO, 5% to 10% of CaO, 1% to 3% of SiO₂, and other inevitable composition.

An overall submerged entry nozzle is used for casting, an insertion depth of the submerged entry nozzle is 10 mm to 15 mm, a mold flux has a slag layer thickness of 10 mm to 20 mm and a consumption rate of 0.15 kg/ton to 0.25 kg/ton.

Each of a stopper rod and the submerged entry nozzle is made of a magnesia carbon material, the stopper rod further includes the following composition in mass percentage: 80% to 85% of MgO, 8% to 12% of C, less than or equal to 1.5% of Al₂O₃, 1% to 4% of SiC, 2% to 3% of SiO₂, and other inevitable impurity composition.

The submerged entry nozzle has an inner wall thickness of 5 mm to 7 mm, and includes the following composition in mass percentage: 75% to 80% of MgO, 6% to 10% of C, 3% to 5% of SiC, 5% to 10% of SiO₂, and other inevitable impurity composition.

**Table 22 Main Parameters of continuous casting tundish for spring steel**

| Steel grade | Parameter | Casting speed, m/min , | Tundis h stable tonnage , t | Toonag e during ladle change, t | Superhea t of tundish, °C | Fluctuation of superheat, °C | Induction heating current, A | Induction heating voltage, V |
|---|---|---|---|---|---|---|---|---|
| 55SiC r | Embodiment 1 | 0.65 | 48 | 45 | 20 | 5 | 1500 | 1800 |
| | Embodiment 2 | 0.60 | 49 | 45 | 30 | 4 | 1700 | 2000 |
| | Embodiment 3 | 0.70 | 47 | 40 | 25 | 5 | 1600 | 1900 |
| 65Mn | Embodiment 4 | 0.66 | 48 | 44 | 26 | 3 | 1800 | 1700 |
| | Embodiment 5 | 0.62 | 49 | 43 | 35 | 4 | 1750 | 1850 |
| | Embodiment 6 | 0.68 | 48 | 42 | 33 | 5 | 1650 | 1750 |

**Table 23 Continuous casting mold and reduction control parameters for spring Steel**

| Steel grad e | Paramete r | Mold water flow rate, NL/m in | Second ary cooling water flow rate, NL/min | Level fluctuati on, mm | Electromag netic stirring current, A | Electromag netic stirring frequency, Hz | Reducti on amount , mm | C segregat ion index of cast billet |
|---|---|---|---|---|---|---|---|---|
| 55Si Cr | Embodi ment 1 | 2750 | 600 | 2.0 | 450 | 6 | 15 | 0.96 |
| | Embodi ment 2 | 2800 | 550 | 1.0 | 480 | 8 | 18 | 1.05 |
| | Embodi ment 3 | 2850 | 580 | 1.5 | 550 | 7 | 20 | 1.03 |
| 65M n | Embodi ment 4 | 2750 | 650 | 1.0 | 500 | 7 | 18 | 0.98 |
| | Embodi ment 5 | 2800 | 600 | 1.2 | 650 | 6 | 22 | 1.02 |
| | Embodi ment 6 | 2800 | 580 | 0.8 | 600 | 8 | 16 | 1.04 |

**Table 24 Main Parameters of continuous casting tundish for cord steel**

| Steel grad e | Parameter | Castin g speed, m/min, | Tundis h stable tonnage , t | Toonag e during ladle change, t | Superhea t of tundish, °C | Fluctuatio n of superheat, °C | Inductio n heating current, A | Inductio n heating voltage, V |
|---|---|---|---|---|---|---|---|---|
| 72A | Embodimen t 7 | 0.66 | 49 | 45 | 25 | 5 | 1500 | 1800 |
| | Embodimen t 8 | 0.62 | 48 | 40 | 20 | 4 | 1700 | 2000 |
| | Embodimen t 9 | 0.60 | 48 | 43 | 30 | 5 | 1600 | 1900 |
| 82A | Embodimen t 10 | 0.66 | 47 | 42 | 30 | 3 | 1800 | 1700 |
| | Embodimen t 11 | 0.68 | 47 | 44 | 35 | 4 | 1750 | 1850 |
| | Embodimen t 12 | 0.70 | 48 | 45 | 40 | 5 | 1650 | 1750 |
| 97A | Embodimen t 13 | 0.60 | 49 | 45 | 40 | 3 | 1800 | 1700 |
| | Embodimen t 14 | 0.62 | 48 | 44 | 45 | 4 | 1750 | 1850 |
| | Embodimen t 15 | 0.65 | 48 | 43 | 30 | 5 | 1650 | 1750 |

**Table 25 Continuous casting mold and reduction control parameters for cord steel**

| Ste el gra de | Paramete r | Mold water flow rate, NL/m in | Second ary cooling water flow rate, NL/min | Level fluctuati on, mm | Electromag netic stirring current, A | Electromag netic stirring frequency, Hz | Reducti on amount , mm | C segregat ion index of cast billet |
|---|---|---|---|---|---|---|---|---|
| 72 A | Embodim ent 7 | 2750 | 550 | 1.0 | 480 | 8 | 16 | 0.95 |
| | Embodim ent 8 | 2780 | 580 | 0.9 | 550 | 7 | 15 | 1.05 |
| | Embodim ent 9 | 2820 | 600 | 1.5 | 450 | 8 | 20 | 1.02 |
| 82 A | Embodim ent 10 | 2750 | 580 | 1.6 | 550 | 6 | 19 | 0.98 |
| | Embodim ent 11 | 2800 | 600 | 1.8 | 600 | 8 | 25 | 1.01 |
| | Embodim ent 12 | 2850 | 620 | 0.7 | 650 | 7 | 18 | 1.04 |
| 97 A | Embodim ent 13 | 3050 | 650 | 1.0 | 600 | 6 | 22 | 1.02 |
| | Embodim ent 14 | 3000 | 630 | 1.3 | 650 | 8 | 30 | 1.01 |
| | Embodim ent 15 | 2950 | 600 | 0.8 | 620 | 8 | 25 | 1.03 |

**Table 26 Main Parameters of continuous casting tundish for cable steel**

| Steel grad e | Parameter | Castin g speed, m/min, | Tundis h stable tonnage , t | Toonag e during ladle change, t | Superhea t of tundish, °C | Fluctuatio n of superheat, °C | Inductio n heating current, A | Inductio n heating voltage, V |
|---|---|---|---|---|---|---|---|---|
| 87B | Embodimen t 16 | 0.68 | 47 | 40 | 30 | 4 | 1600 | 1900 |
| | Embodimen t 17 | 0.70 | 48 | 44 | 35 | 5 | 1800 | 1800 |
| | Embodimen t 18 | 0.68 | 49 | 43 | 43 | 5 | 1650 | 1950 |
| 92Si | Embodimen t 19 | 0.65 | 48 | 44 | 45 | 4 | 1750 | 2000 |
| | Embodimen t 20 | 0.60 | 49 | 45 | 36 | 3 | 1700 | 1950 |
| | Embodimen t 21 | 0.66 | 48 | 42 | 40 | 5 | 1650 | 1750 |

**Table 27 Continuous casting mold and reduction control parameters of Cable Steel**

| Ste el gra de | Paramete r | Mold water flow rate, NL/m in | Second ary cooling water flow rate, NL/min | Level fluctuati on, mm | Electromag netic stirring current, A | Electromag netic stirring frequency, Hz | Reducti on amount , mm | C segregat ion index of cast billet |
|---|---|---|---|---|---|---|---|---|
| 87B | Embodim ent 16 | 2850 | 500 | 1.0 | 580 | 7 | 30 | 0.97 |
| | Embodim ent 17 | 2900 | 550 | 1.5 | 450 | 6 | 26 | 1.03 |
| | Embodim ent 18 | 2950 | 620 | 2.0 | 550 | 8 | 22 | 1.05 |
| 92S i | Embodim ent 19 | 3050 | 630 | 0.9 | 550 | 7 | 28 | 0.99 |
| | Embodim ent 20 | 3000 | 650 | 1.6 | 600 | 8 | 25 | 1.02 |
| | Embodim ent 21 | 2950 | 600 | 0.8 | 660 | 7 | 26 | 1.03 |

### Step 6: Cogging and grinding

The continuously cast billet is heated in a cogging reheating furnace and undergoes soaking and heat preservation, a billet temperature is controlled to be 1100°C to 1200°C, and an initial rolling temperature is controlled to be 1040°C to 1180°C; a rolled billet is obtained after cogging and rolling; the rolled billet is subjected to magnetic particle inspection, followed by full surface grinding; and for a position with an apparent flaw detection defect on the surface, spot grinding is carried out additionally, with an average grinding depth of ≥0.5 mm.

**In** a case of controlling an atmosphere in the reheating furnace, the rolled billet after coating spraying is heated in a steel-rolling reheating furnace and undergoes soaking and heat preservation, and the heating time the billet rolling temperature and the initial rolling temperature in the steel rolling reheating furnace are controlled. In percent by volume, a total content of H₂O and O₂ in atmosphere composition in the reheating furnace is ≤2.5%.

**Table 28 Main process parameters of cogging and grinding for spring steel**

| Steel grade | Parameter | Soaking section time, min | Billet temperature, °C | Initial rolling temperature, °C | Average grinding depth, ≥mm |
|---|---|---|---|---|---|
| 55SiCr | Embodiment 1 | 350 | 1150 | 1120 | 1.5 |
| | Embodiment 2 | 300 | 1180 | 1140 | 1.3 |
| | Embodiment 3 | 330 | 1170 | 1130 | 1.2 |
| 65Mn | Embodiment 4 | 230 | 1170 | 1140 | 0.8 |
| | Embodiment 5 | 250 | 1200 | 1160 | 0.5 |
| | Embodiment 6 | 280 | 1190 | 1150 | 1.0 |

**Table 29 Main process parameters of cogging and grinding for cord steel**

| Steel grade | Parameter | Soaking section time, min | Billet temperature, °C | Initial rolling temperature, °C | Average grinding depth, ≥mm |
|---|---|---|---|---|---|
| 72A | Embodiment 7 | 180 | 1100 | 1070 | 0.5 |
| | Embodiment 8 | 200 | 1140 | 1110 | 0.7 |
| | Embodiment 9 | 220 | 1120 | 1090 | 0.6 |
| 82A | Embodiment 10 | 200 | 1120 | 1080 | 0.7 |
| | Embodiment 11 | 250 | 1140 | 1100 | 0.9 |
| | Embodiment 12 | 230 | 1150 | 1090 | 0.8 |
| 97A | Embodiment 13 | 250 | 1180 | 1040 | 0.6 |
| | Embodiment 14 | 280 | 1200 | 1170 | 1.0 |
| | Embodiment 15 | 300 | 1170 | 1150 | 1.2 |

**Table 30 Main process parameters of cogging and grinding for cable steel**

| Steel grade | Parameter | Soaking section time, min | Billet temperature, °C | Initial rolling temperature, °C | Average grinding depth, ≥mm |
|---|---|---|---|---|---|
| 87B | Embodiment 16 | 250 | 1130 | 1090 | 0.8 |
| | Embodiment 17 | 220 | 1150 | 1110 | 0.9 |
| | Embodiment 18 | 200 | 1140 | 1100 | 0.7 |
| 92Si | Embodiment 19 | 350 | 1190 | 1050 | 1.5 |
| | Embodiment 20 | 320 | 1200 | 1180 | 1.2 |
| | Embodiment 21 | 300 | 1180 | 1170 | 1.0 |

### Step 7. Rolling and air cooling

The 140 mm×140 mm rolled billet obtained from cogging is ground, and then a high-temperature-resistant coating is sprayed on a surface of the rolled billet, with a coating thickness of 0.3 mm to 1.5 mm.

**A** rolled wire obtained in the high-speed wire rod rolling procedure is subjected to temperature-controlled air cooling, and a wire laying temperature of an air cooling line is controlled at 820°C to 900°C.

The high-temperature coating includes CaO, SiO₂, Al₂O₃, MgO, ZrO₂, C, as well as small amounts of alkali metal oxides, inorganic binders, surfactants, and the like.

The bloom is cogged and rolled into a billet with a cross-section of 140 mm×140 mm, followed by flow inspection and grinding, heating in a reheating furnace, rolling, and temperature-controlled cooling on a Stelmor air-cooling line, so that an obtained wire rod is free from surface defects such as seams, scabs, and scratches, and there is no fully decarburized layer on a surface thereof.

A wire rod prepared from the high-purity high-carbon steel wire includes a high-quality cord steel wire rod with a C content of ≤0.87% for drawing a fine wire with a diameter of 0.1 mm or more and a high-quality diamond wire rod with a C content is more than 0.87% and less than or equal to 1.0% for drawing a fine wire with a diameter of 0.05 mm or more.

A 1600-2400 MPa grade spring steel and a 1800-2200 MPa grade cable steel prepared from the high-purity high-carbon steel wire are provided.

**Table 31 Main process parameters in rolling and air cooling for spring steel**

| Steel grade | Parameter | Coating thicknes s, min | Billet temperatur e, °C | Initial rolling temperatur e, °C | Entry temperatu re of finish rolling, °C | Exit temperatu re of finish rolling, °C | Wire laying temperatur e, °C |
|---|---|---|---|---|---|---|---|
| 55SiC r | Embodime nt 1 | 1.5 | 1030 | 910 | 840 | 1010 | 840 |
| | Embodime nt 2 | 1.3 | 1080 | 970 | 890 | 1030 | 860 |
| | Embodime nt 3 | 1.4 | 1050 | 940 | 875 | 1020 | 850 |
| 65Mn | Embodime nt 4 | 1.0 | 1080 | 980 | 930 | 1010 | 835 |
| | Embodime nt 5 | 1.1 | 1130 | 1010 | 950 | 1030 | 850 |
| | Embodime nt 6 | 0.8 | 1100 | 995 | 920 | 1000 | 820 |

**Table 32 Main process parameters in rolling and air cooling for cord Steel**

| Steel grad e | Parameter | Coating thicknes s, min | Billet temperatur e, °C | Initial rolling temperatur e, °C | Entry temperatur e of finish rolling, °C | Exit temperatur e of finish rolling, °C | Wire laying temperatur e, °C |
|---|---|---|---|---|---|---|---|
| 72A | Embodime nt 7 | 0.3 | 1110 | 1005 | 920 | 1020 | 870 |
| | Embodime nt 8 | 0.5 | 1130 | 1020 | 950 | 1040 | 890 |
| | Embodime nt 9 | 0.7 | 1090 | 990 | 935 | 1030 | 880 |
| 82A | Embodime nt 10 | 0.9 | 1125 | 1015 | 935 | 1035 | 915 |
| | Embodime nt 11 | 0.6 | 1150 | 1030 | 950 | 1050 | 925 |
| | Embodime nt 12 | 0.8 | 1100 | 1000 | 920 | 1020 | 905 |
| 97A | Embodime nt 13 | 1.5 | 1145 | 1045 | 945 | 1040 | 900 |
| | Embodime nt 14 | 1.3 | 1160 | 1060 | 960 | 1050 | 920 |
| | Embodime nt 15 | 1.4 | 1130 | 1030 | 930 | 1030 | 880 |

**Table 33 Main process parameters in rolling and air cooling for cable steel**

| Steel grad e | Parameter | Coating thicknes s, min | Billet temperatur e, °C | Initial rolling temperatur e, °C | Entry temperatur e of finish rolling, °C | Exit temperatur e of finish rolling, °C | Wire laying temperatur e, °C |
|---|---|---|---|---|---|---|---|
| 87B | Embodime nt 16 | 1.3 | 1135 | 1025 | 940 | 1010 | 870 |
| | Embodime nt 17 | 1.2 | 1150 | 1035 | 950 | 1020 | 880 |
| | Embodime nt 18 | 1.0 | 1120 | 1015 | 930 | 990 | 880 |
| 92Si | Embodime nt 19 | 1.5 | 1170 | 1055 | 950 | 1020 | 880 |
| | Embodime nt 20 | 1.3 | 1190 | 1070 | 960 | 1030 | 890 |
| | Embodime nt 21 | 1.4 | 1150 | 1040 | 940 | 1000 | 870 |

The present disclosure can implement the following:
(1) KR and the converter can reduce S content to a low level, thereby avoiding the formation of a high-basicity slag system during the refining for desulfurization. As desulfurization involves intense slag-metal reactions that alter an inclusion composition system, precise control of the S content in the KR and converter stages can achieve accurate control of inclusion composition types.
**(2)** The converter adopts a double-slag process. By precisely controlling a bath temperature, slag basicity, oxidizability, and bottom-blowing stirring in the early stage of blowing, low-phosphorus semi-steel hot metal is obtained. A high-basicity and high-oxidizability slag is further formed. In particular, through precise addition of pellets during the blowing, the oxidizability of the slag is controlled throughout the entire process to avoid the problem of phosphorus reversion, thereby obtaining low-phosphorous molten steel.
(3) During converter tapping, carbon powder and metallic manganese are used for partial deoxidation to reduce nitrogen pickup by the molten steel. In addition, MnO- based inclusions are predominantly formed. Under the deep vacuum conditions of the RH process, silicon carbide, ultra- pure silicon, and carbon powder are used for deoxidation and alloying, which can reduce the total amount of inclusions generated, decrease the pumping capacity of RH, weaken the stirring intensity of the molten steel, reduce the reduction of MnO inclusions by Si, thereby obtaining SiO₂- MnO inclusions with a high MnO content. Combined with control of the alloys, refractory materials, and low- basicity slag system, the contents of high- melting-point composition such as CaO, Al₂O₃, and MgO in the inclusions are further reduced.
(4) A non-symmetric flow rate stirring mode with a limited maximum flow rate is adopted throughout the entire refining process. Dead zones caused by molten steel impingement are reduced, molten steel circulation is promoted, temperature and composition homogenization are accelerated, the duration of intense slag- metal reactions is shortened, inclusions introduced by slag entrainment are reduced, and the efficient removal of inclusions are facilitated at the same time.
(5) Control of auxiliary materials such as ladle, vacuum vessel, and continuous casting refractory materials reduces the sources of alumina- type inclusions, improves the quality of refractory materials, and decreases erosion of refractory material that may otherwise form large- sized exogenous brittle inclusions. In addition, the RH process adopts a variable circulation intensity approach to remove inclusions. In the early stage, high vacuum and high lift gas flow rate are used to remove low- melting- point acidic inclusions, which exhibit a certain degree of erosion toward the refractory materials. Low- carbon refractory materials are employed to mitigate deoxidation- induced erosion. In the middle and late stages, weak circulation stirring is applied to reduce erosion of the refractory materials and promote the floating of large- sized silicate- based composite inclusions formed by early-stage erosion. Combined with soft stirring after breaking vacuum, as well as killing and electromagnetic stirring during continuous casting, the floating of inclusions is further enhanced.
(6) Continuous casting employs narrow- range superheat control, matching control of alloying elements with superheat, and constant casting speed technology to achieve precise segmented reduction control. Segregation of various elements in the cast billet can be mitigated, thereby reducing the formation of precipitate inclusions. In addition, internal cracking and other problems caused by improper distribution of applied stress during reduction can be avoided.
(7) During cogging and rolling, a high-temperature and long-time heating technology is adopted to promote uniform diffusion of elements and eliminate the problems of element segregation and the like. In addition, integrated with the full grinding of the billet the application technology of a novel coating material, the surface decarburization of the wire rod can be reduced. By optimizing a controlled cooling process, an excellent wire rod with excellent microstructure and properties can be obtained.

The technical means disclosed by the solution of the present disclosure are not limited to the technical means disclosed by the foregoing technical means, and further include the technical solutions consisting of any combination of the foregoing technical features.

Inspired by the foregoing ideal embodiments according to the present disclosure, through the above description, those skilled in the art can make various changes and modifications within the scope without departing from the technical concept of the present disclosure.

## Claims

1. A method for manufacturing a high-purity high-carbon steel wire, wherein production is carried out according to the following technological processes: hot metal pretreatment, converter smelting, RH (Ruhrstahl-Heraeus) vacuum treatment, bloom continuous casting, cogging and grinding, high-speed wire-rod rolling, Stelmor air cooling, and finished wire rod obtaining, and the method specifically comprises the following steps:
Step 1: carrying out KR (Kanbara Reactor) hot metal pretreatment to low-sulfur hot metal, and charging the low-sulfur hot metal into a converter;
Step 2: carrying out converter smelting with a converter charge of 145±5 t and a hot metal ratio of 80% to 90%, wherein clean scrap is selected for smelting, and the converter adopts a double-slag dephosphorization process;
Step 3: during converter tapping, at the start of tapping, adding 30% to 40% of low-nitrogen carburizer into a ladle at first, and adding 20% to 30% of metallic manganese for pre-deoxidation, completing tapping after the added low-nitrogen carburizer and metallic manganese are fully dissolved into molten steel and no carbon powder particles float on the surface, and then adding silicon carbide and a synthetic slag to ladle slag surface in sequence to deoxidize the slag surface and form slag;
during converting tapping, maintaining ladle bottom blowing throughout the entire process, wherein in dual bottom blowing of the ladle, one porous plug has a maximum flow rate of 600 NL/min to 800 NL/min, and the other porous plug has a flow rate of 30% to 50% of the maximum flow rate, the two porous plugs are arranged on the bottom of the ladle at an angle of 135 degrees, located at a position 55% of a radius from the center of the ladle, and configured to blow argon into the molten steel to stir the molten steel and the slag;
upon completion of converter tapping, adding silicon carbide to deoxidize the ladle slag, with at an addition amount of 0.5 kg/t to 1.5 kg/t, and after the silicon carbide is added, adding a synthetic slag for slag formation, with an addition amount of 8 kg/t to 12 kg/t; controlling dual bottom blowing flow rates of the ladle at 150 NL/min to 250 NL/min after the synthetic slag is added, and transporting the ladle to RH for treatment after the synthetic slag is evenly spread;
Step 4: RH furnace refining, enabling a RH arrival temperature to be ≥1590°C, C content to be ≥0.2%, Mn content to be 0.15-0.35%, and oxygen content to be ≤0.020%; carrying out rapid evacuation treatment upon arrival at a RH station; adding silicon carbide for deoxidation, taking a sample for composition test, and based on a composition test result and a composition requirement of a smelted steel grade, selecting one or more of low-nitrogen carburizer, ultra-pure silicon, metallic manganese, ferrochrome, and ferrovanadium for alloying; after the composition meets standards, reducing a pumping capacity of a RH vacuum system by 40% to 60%, increasing a pressure in a vacuum chamber, reducing a lift gas flow rate to 80 Nm³/min to 100 Nm³/min, and after carrying out net circulation for ≥5 min, breaking vacuum, initiating bottom-blowing soft stirring of the ladle, transporting the ladle to a continuous casting platform to stand for 10 min and more, and then starting casting;
during rapid evacuation treatment upon arrival at the RH station, controlling an operating pressure of the vacuum chamber to be ≤1 mbar, the lift gas flow rate to be 150 Nm³/min to 200 Nm³/min, and deep vacuum treatment time to be ≥15 min; and after the composition meets the standards, increasing the pressure in the vacuum chamber pressure to above 50 mbar;
in Step 4, after vacuum breaking in RH, controlling soft stirring time to be ≥6 min, the maximum flow rate of one of the dual porous plugs to be 60 NL/min to 80 NL/min, and the flow rate of the other porous plug to be 40% to 50% of the maximum flow rate;
Step 5: carrying out bloom continuous casting;
Step 6: carrying out cogging and grinding to improve surface quality; and
Step 7: carrying out rolling and air cooling to control cooling intensity and improve structure and properties.

2. The method for manufacturing a high-purity high-carbon steel wire according to claim 1, wherein step 2 comprises the following steps: adopting intensive bottom-blowing stirring in an early stage of converter blowing, with a high lance position and a low oxygen flow rate, adopting a medium-basicity slag system with basicity of 1.8 to 2.2; adding pellets to control a T.Fe content in the slag to be ≥25%; stopping oxygen blowing upon completion of early-stage blowing, controlling a temperature to be 1380°C to 1430°C, carrying out bottom-blowing stirring for more than 3 min until a P content is ≤0.016%, followed by slag removal; after the slag removal is completed, continuing blowing with a low lance position and a high oxygen supply flow rate; adding lime to form a high-basicity slag system, and adding pellets to control a minimum T.Fe to be ≥15% during blowing; at the end of blowing, controlling the temperature to be ≥1650°C, the T.Fe content to be ≥25%, and the basicity to be ≥6; and carrying out slag removal at first, and upon completing the slag removal, tapping while retaining the slag with a slide gate.

3. The method for manufacturing a high-purity high-carbon steel wire according to claim 1, wherein in step 5, the bloom has a cross-section of 300 mm×390 mm, protective casting is implemented throughout the entire continuous casting process, a low-basicity and low-alumina tundish covering flux is adopted, and tundish electromagnetic induction heating equipment is configured to control a superheat fluctuation of the molten steel in the tundish to be ≤5°C, with a tundish induction heating current of 1500 A to 1800 A and a voltage of 1600 V to 2000 V; when a carbon content in the steel is 0.5%≤C<0.8%, the superheat of molten steel is controlled at 20°C to 35°C; and when a carbon content in the steel is that 0.8%≤C<1.0%, the superheat of the molten steel is controlled at 30°C to 45°C, a tundish tonnage is maintained at 48±1 tons, and the tonnage during ladle change is controlled at 40 tons to 45 tons.

4. The method for manufacturing a high-purity high-carbon steel wire according to claim 1, wherein in step 5, the mold electromagnetic stirring is carried out with a current of 450 A 650 A and a frequency of 6 Hz to 8 Hz, a mold water flow rate is set to 2750 NL/min to 3050 NL/min, a secondary cooling segment water flow rate is set to 550 NL/min to 650 NL/min, and a mold level fluctuation is set to ≤2 mm; and continuous casting is carried out at a constant casting speed, and the continuous casting speed is controlled at 0.6 m/min to 0.7 m/min.

5. The method for manufacturing a high-purity high-carbon steel wire according to claim 4, wherein in step 5, a solid fraction fs at the solidification center of a continuously cast billet is divided into four ranges, when 0.1≤fs<0.3, a reduction ratio accounts for 10% to 15%; when 0.3≤fs<0.5, a reduction ratio accounts for 20% to 30%; when 0.5≤fs<0.8, a reduction ratio accounts for 50% to 60%; when 0.8≤fs<1, a reduction ratio accounts for 10% to 20%; and a total reduction amount is controlled at 15 mm to 30 mm, thereby obtaining a cast billet with C segregation index of 0.95 to 1.05.

6. The method for manufacturing a high-purity high-carbon steel wire according to claim 1, wherein in step 6, during cogging and grinding, the continuously cast billet is heated in a cogging reheating furnace and undergoes soaking and heat preservation, a billet temperature is controlled to be 1100°C to 1200°C, and an initial rolling temperature is controlled to be 1040°C to 1180°C; a rolled billet is obtained after cogging and rolling; the rolled billet is subjected to magnetic particle inspection, followed by full surface grinding; and for a position with an apparent flaw detection defect on the surface, spot grinding is carried out additionally, with an average grinding depth of ≥0.5 mm; and
during coating spraying of the rolled billet, a high-temperature-resistant coating is sprayed onto the surface of the ground rolled billet, with a thickness of 0.3 mm to 1.5 mm.

7. The method for manufacturing a high-purity high-carbon steel wire according to claim 6, wherein in step 6, in a case of controlling an atmosphere in the reheating furnace, the rolled billet after coating spraying is heated in a steel-rolling reheating furnace and undergoes soaking and heat preservation, a temperature of the rolled billet in the steel-rolling reheating furnace is controlled at 1030°C to 1190°C, an initial rolling temperature is controlled at 910°C to 1170°C, a finish rolling entry temperature is controlled at 840°C to 960°C, and a finish rolling exit temperature is controlled at 990°C to 1050°C; and in percent by volume, a total content of H₂O and O₂ in atmosphere composition in the reheating furnace is ≤2.5%.

8. The method for manufacturing a high-purity high-carbon steel wire according to claim 1, wherein in step 7, a rolled wire obtained in a high-speed wire rod rolling procedure is subjected to temperature-controlled air cooling, and a wire laying temperature of an air cooling line is controlled at 820°C to 925°C.

9. The method for manufacturing a high-purity high-carbon steel wire according to claim 1, wherein a KR arrival temperature is ≥1380°C, and in the hot metal, an S content is ≤0.045%, a C content is 4.1% to 4.6%, an Si content is 0.25% to 0.60%, a Ti content is ≤0.03%, a P content is ≤0.11%, with the balancing being Fe and other inevitable impurity elements; upon arrival at a KR station, a blast furnace slag is skimmed with a slag skimming rate of ≥95%; then, a desulfurizing agent is added for desulfurization, and after desulfurization, slag skimming is carried out again with a slag skimming rate of ≥95%; subsequently, the desulfurizing agent is added for the second desulfurization, with a slag skimming rate of ≥ 98%; and a KR departure temperature is controlled to be ≥1330°C, and a departure S content is controlled to be ≤0.0008%.

10. The method for manufacturing a high-purity high-carbon steel wire according to claim 1, wherein the clean scrap used by the converter comprises composition as follows: less than or equal to 0.015% of P, less than or equal to 0.0050% of S, less than or equal to 0.01% of Ti, and conventional elements such as C, Si, Al, Mn, Fe.

11. The method for manufacturing a high-purity high-carbon steel wire according to claim 1, wherein at the end of converter blowing, a C content is 0.03% to 0.07%, an O content is 0.035% to 0.075%, a P content is ≤0.008%, and a tapping weight of the converter is 135±5 t.

12. The method for manufacturing a high-purity high-carbon steel wire according to claim 1, wherein the low-carbon nitrogen carburizer added during converter tapping comprises less than or equal to 0.045% of N, with the balance being C and inevitable impurity elements;
the metallic manganese comprises more than or equal to 99% of Mn, less than or equal to 0.003% of Ti, less than or equal to 0.005% of Al, less than or equal to 0.0065% of P, less than or equal to 0.0035% of S, with the balance being iron and inevitable impurity elements; and
the silicon carbide comprises more than or equal to 98% of SiC, and other inevitable impurity elements.

13. The method for manufacturing a high-purity high-carbon steel wire according to claim 1, wherein the synthetic slag added during converter tapping comprises composition as follows: 45% to 55% of CaO, 20% to 30% of SiO₂, 5% to 10% of CaF₂, 1% to 3% of MnO, less than or equal to 3% of MgO, less than or equal to 1.5% of Al₂O₃, and other inevitable impurity composition, and has a basicity of 1.5 to 2.0; and in phase composition, monocalcium silicate accounts for 35% to 45%, dicalcium silicate accounts for 15% to 25%, and the others are CaO, CaF₂, MnO, and inevitable phases.

14. The method for manufacturing a high-purity high-carbon steel wire according to claim 1, wherein the low-carbon nitrogen carburizer added during RH vacuum treatment comprises less than or equal to 0.045% of N, with the balance being C and inevitable impurity elements;
the metallic manganese comprises more than or equal to 99% of Mn, less than or equal to 0.003% of Ti, less than or equal to 0.005% of Al, less than or equal to 0.0065% of P, less than or equal to 0.0035% of S, with the balance being iron and inevitable impurity elements; and
the silicon carbide comprises more than or equal to 98% of SiC, and other inevitable impurity elements;
the ultra-pure silicone comprises 80% to 85% of Si, less than or equal to 0.0035% of Al, less than or equal to 0.001% of Ti, less than or equal to 0.005% of P, less than or equal to 0.0025% of S, with the balance being iron and inevitable impurity elements;
the ferrochrome comprises 55% to 60% of Cr, less than or equal to 1.8% of C, less than or equal to 0.006% of S, less than or equal to 0.013% of P, with the balance being iron and inevitable impurity elements; and
the ferrovanadium comprises 45% to 50% of V, less than or equal to 1.6% of C, less than or equal to 0.005% of S, less than or equal to 0.012% of P, with the balance being iron and inevitable impurity elements.

15. The method for manufacturing a high-purity high-carbon steel wire according to claim 1, wherein a ladle brick used in step 3 is a magnesia-carbon brick, which comprises less than or equal to 3.0% of magnesium aluminate spinel, less than or equal to 3% of C, with the balance being inevitable impurity composition;
a refractory material used for a dipping tube and a bottom tank of a RH vacuum furnace in step 4 is an ultra-low-carbon magnesite-chrome brick, which comprises less than or equal to 1.5% of C, 85% to 95% of MgO, 5% to 12% of Cr₂O₃, less than or equal to 3.0% of magnesium aluminate spinel, and other inevitable impurity composition.

16. The method for manufacturing a high-purity high-carbon steel wire according to claim 3, wherein the low-basicity and low-alumina tundish covering flux for continuous casting comprises main composition as follows: 40%-50% of CaO, 30% to 40% of /SiO₂, 3% to 6% of CaF₂, less than or equal to 2% of Al₂O₃, 3% to 6% of MgO, and other inevitable composition; and
a magnesia spraying material for an inner wall of the tundish comprises composition as follows: more than or equal to 80% of MgO, 5% to 10% of CaO, 1% to 3% of SiO₂, and other inevitable composition.

17. The method for manufacturing a high-purity high-carbon steel wire according to claim 4, wherein in step 5, an overall submerged entry nozzle is used for casting, an insertion depth of the submerged entry nozzle is 10 mm to 15 mm, a mold flux has a slag layer thickness of 10 mm to 20 mm and a consumption rate of 0.15 kg/ton to 0.25 kg/ton;
each of a stopper rod and the submerged entry nozzle is made of a magnesia carbon material, the stopper rod further comprises the following composition in mass percentage: 80% to 85% of MgO, 8% to 12% of C, less than or equal to 1.5% of Al₂O₃, 1% to 4% of SiC, 2% to 3% of SiO₂, and other inevitable impurity composition; and
the submerged entry nozzle has an inner wall thickness of 5 mm to 7 mm, and comprises the following composition in mass percentage: 75% to 80% of MgO, 6% to 10% of C, 3% to 5% of SiC, 5% to 10% of SiO₂, and other inevitable impurity composition.

18. The method for manufacturing a high-purity high-carbon steel wire according to claim 1, wherein in step 6, a coating is sprayed for protection before the rolled billet enters the reheating furnace, wherein the coating has a thickness of 0.3 mm to 1.5 mm, and the high-temperature coating comprises CaO, SiO₂, Al₂O₃, MgO, ZrO₂, C, as well as small amounts of alkali metal oxides, inorganic binders, and surfactants.

19. The method for manufacturing a high-purity high-carbon steel wire according to claim 3, wherein the bloom is cogged into a billet with a cross-section of 140 mm×140 mm, and is subjected to flow inspection and grinding, heating in a reheating furnace, rolling, and controlled cooling on a Stelmor air-cooling line to obtain a wire rod that is free from surface defects such as a fold, a scab, and a scratch, and has no fully decarburization layer on surface thereof.

20. High-purity high-carbon steel wire manufactured according to the method according to any one of claims 1 to 19.

21. A wire rod, wherein the wire rod is prepared from the high-purity high-carbon steel wire according to claim 20, the wire rod comprises a high-quality cord steel wire rod with a C content of ≤0.87% for drawing a fine wire with a diameter of 0.1 mm or more and a high-quality diamond wire rod with a C content is more than 0.87% and less than or equal to 1.0% for drawing a fine wire with a diameter of 0.05 mm or more.

22. A 1600-2400 MPa grade spring steel and a 1800-2200 MPa grade cable steel prepared from the high-purity high-carbon steel wire according to claim 20.

23. The high-purity high-carbon steel wire according to claim 20, wherein the high-purity high-carbon steel wire, in addition to alloying elements and Fe element, further comprises the following chemical composition in mass percentage: 0.5% to 1.0% of C, less than or equal to 0.008% of P, less than or equal to 0.0025% of S, less than or equal to 0.0010% of T.O, less than or equal to 0.0020% of N, less than or equal to 0.0002% of H, less than or equal to 0.0010% of Alt, and less than or equal to 0.0005% of Ti.

24. The high-purity high-carbon steel according to claim 23, wherein in the high-carbon steel wire rod, a mass content of inclusions other than those of the SiO₂-MnO type is ≤ 20%, a number density of inclusions larger than 1 µm is ≤3.5 particles/mm², and a number density of inclusions larger than 5 µm is ≤0.06 particles/mm²; the maximum transverse size of inclusions is ≤12 µm, longitudinal inclusions has a maximum width of ≤10 µm and a length of ≤25 µm; the size of brittle inclusions is ≤3 µm; a carbon segregation index of the cast billet is 0.95 to 1.05, and a carbon segregation index of the wire rod is ≤1.05.
